# EUROPEAN PATENT SPECIFICATION

(11) **EP 0 559 837 B1**
(45) Date of publication and mention of the grant of the patent: **25.10.1995**
(21) Application number: 92904074.9
(22) Date of filing: 20.11.1991
(51) Int. Cl.: C11D 17/00, C11D 1/04, C11D 1/08, C11D 10/04

(54) **SHAPED SOLID MADE WITH A RIGID, INTERLOCKING MESH OF NEUTRALIZED CARBOXYLIC ACID**
MIT EINER AUS NEUTRALISIERTER,CARBONSÄURE-FESTEN, INEINANDERGREIFENDEN MASCHE HERGESTELLTER GEFORMTER FESTKÖRPER
SOLIDE FACONNE COMPOSE D'UNE MAILLE RIGIDE A EMBOITEMENTS D'ACIDE CARBOXYLIQUE NEUTRALISE

(30) Priority: 26.11.1990 US 617827; 01.11.1991 US 782956
(43) Date of publication of application: 15.09.1993
(73) Proprietor: THE PROCTER & GAMBLE COMPANY, Cincinnati, Ohio 45202 (US)
(72) Inventor: KACHER, Mark, Leslie, Mason, OH 45040 (US); TANERI, James, Eden, Neenah, Wisconsin 54956 (US); CAMDEN, James, Berger, West Chester, Ohio 45069-1594 (US); VEST, Paul, Edward, Cincinnati, OH 45255 (US); BOWLES, Sylvia, Jean, Cincinnati, OH 45231 (US)
(74) Representative: Brooks, Maxim Courtney
(86) International application number: US9108733
(87) International publication number: WO9209679

(56) References cited:
- EP-A- 0 294 010
- EP-A- 0 308 190
- WO-A-88/06617
- DE-A- 2 132 035
- FR-A- 2 518 568
- US-A- 3 226 329
- US-A- 3 926 828
- US-A- 4 165 293
- US-A- 4 396 521

## Description

This invention relates to neutralized carboxylic acid shaped solid compositions, particularly cleansing bars, cakes, soap bars, synbars and the like.

Products made in the form of shaped solids, cakes and bars are numerous. Cleansing bars are well known in the art.

Cleansing bars with reduced bar smear are reported in the art. E.g., US-A-2,988,511, Mills, issued June 13, 1961, discloses a low smearing bar.

Bar smear, also referred to as bar sloth, is the soft solid or mush that forms at the surface of a bar when submerged in water and is regarded by consumers as messy, unattractive, and uneconomical.

Products made in the form of shaped solids, cakes and bars are numerous. E.g., certain high moisture and low smear personal cleansing bars are disclosed in US-A-4,606,839 Harding, issued Aug. 19, 1986. Harding uses coconut and/or palm kernel oil soap.

One only has to examine a used personal cleansing bars in their bathroom to see that there is still a need for improved cleansing bars with little or no smear.

The formation of rigid, soap curd fibers of sodium laurate is reported by L. Marton et al. in a 1940 Journal of American Chemical Society (Vol. 63, pp. 1990-1993). The report does not teach a utility for the soap curd. Shaped solids, as defined herein, are not disclosed by Marton et al.

JP-A-7030-798, July 30, 1980, discloses transparent solid framed or molded soap bar in which fatty acids constituting the soap component are myristic, palmitic, and stearic acids. A transparent soap is described in which at least 90 wt.% of the fatty acids which constitute the soap component are myristic acid, palmitic acid, and stearic acid. The product is reported as a transparent, solid soap having good frothing and solidifying properties, good storage stability, and a low irritant effect on human skin. The process and transparent bar soap composition exemplified in JP-A-7030-798 do not appear to contain synthetic surfactant.

It is also difficult to produce firm, non-sticky bars that contain relatively high levels (15-40%) of moisture (especially in the presence of most synthetic surfactants), hygroscopic surfactants and/or higher levels of non-solids and soft solids, such as water-soluble polyols and hydrocarbon greases.

The invention provides a cleansing bar comprising a shaped, solid three-dimensional skeleton structure comprising: a relatively rigid, interlocking mesh of neutralized crystalline carboxylic acid, wherein the rigid, interlocking mesh of neutralized carboxylic acid, preferably comprises sodium soap fibers. Some cleansing bars which comprise surprisingly large amounts of water and other liquids while maintaining their rigidity and excellent smear properties; even when allowed to soak overnight in water.

Figures 1-8 show magnified views of bar samples of the present invention. Figures 9 and 10 show magnified views of two different conventional soap bars.

The Scanning Electron Microscopy (SEM) sample preparation involves fracturing a shaped solid with simple pressure to obtain a fresh surface for examination. The fractured sample is reduced in size (razor blade) to approximately a 10 mm x 15 mm rectangle with a thickness of about 5 mm. The sample is mounted on an aluminum SEM stub using silver paint adhesive. The mounted sample is coated with approximately 300 angstroms of gold/palladium in a Pelco sputter coater. Prior to coating, the sample is subjected to vacuum for a period of time which is sufficient to allow sufficient loss of bar moisture assuring acceptable coating quality. After coating, the sample is transferred to the SEM chamber and examined under standard SEM operating conditions with an Hitachi Model S570 Scanning Electron Microscope in order to see the skeletal (core) frame.

FIGS. 1 and 2 are copies of photographs of a highly enlarged skeleton core structure comprising a rigid, interlocking mesh of elongated neutralized carboxylic acid crystalline fibers. More specifically FIGS. 1 and 2 are elongated C₁₂ sodium soap fibers, enlarged respectively at 5000X and 2500X magnifications. The structure of FIGS. 1 and 2 are made with 5% soap; 94% water; and 1% sodium chloride. See Example 10 in Table 7 herein. Note that larger fibers in the interlocking mesh can be composed of smaller fibers. Also, note the "void" spaces. See FIG. 2.

FIGS. 3, 4 and 5 are copies of photographs of a skeleton structure made with 25% sodium C₁₂ soap; 74% water; and 1% sodium chloride. The crystalline fiber-like structure is shown respectively at 3000X, 5000X and 1000X magnifications.

FIG. 6 is a copy of a photograph of a skeleton structure made with 20% disodium salt of 1,12-dodecanedioic acid. The crystalline fiber-like structure is shown at 2000X magnification. See Example 26.

FIG. 7 is a copy of a photograph of a skeleton (core) structure comprising crystalline lithium neutralized C₁₄ carboxylic acid mesh, shown at 1500X magnification. See Example 27.

FIG. 8 is a copy of a photograph of a cleansing bar (Example I hereinbelow) comprising: coated C₁₄₋₁₆ sodium soap fibers. The fibers are coated and/or commingled with the other bar components. The magnification is 1500X.

FIG. 9 shows a sample of a market IVORY (RTM) freezer bar made with sodium/potassium coconut/tallow soap at 1000X on the scale. The air in the IVORY (RTM) bar soap makes it float.

FIG. 10 shows a sample of a market NEUTROGENA (RTM) transparent bar at 1500X.

In FIGS. 1 and 2, the samples are first melted on a hot plate and recooled on a glass slide. The other samples, FIGS. 3-10, are samples of original shaped solid structures or the conventional bar prepared as set out herein.

The invention provides a cleansing bar comprising a shaped solid comprising two or more phases. One phase is a crystalline skeleton structure comprising a rigid interlocking, open, three-dimensional mesh of neutralized carboxylic acid elongated crystals. The other essential phase is an aqueous phase which is soft or flowable at 25°C.

More specifically, the skeleton structure is a relatively rigid, interlocking, open, three-dimensional mesh of neutralized mono- and/or di-carboxylic acid elongated crystals.

The terms: skeleton structure, skeletal structure, core, and skeleton frame are often used interchangeably herein.

The term "shaped solids" as used herein includes forms such as bars, cakes and the like. The term "bar" as used herein includes the same unless otherwise specified.

The term "mesh" as used herein means an interlocking crystalline skeleton network with voids or openings when viewed under magnification by scanning electron microscopy.

In another respect, the present invention provides an improved cleansing bar which is comprised of said skeleton structure. Some shaped solids are in the form of cleansing bars which contain surprisingly high levels of said aqueous phase comprising water, other liquids and soft materials. Notwithstanding the presence of relatively large levels of an aqueous phase, the preferred bars of the present invention maintain their rigidity and excellent smear properties, even when allowed to soak overnight in water. While not being bound to any theory, the shaped solid comprising these phases is similar to a relatively rigid wet sponge.

The crystalline phase comprises crystals in the form of either interlocking platelets and/or fibers, preferably fibers. Preferably said fibers are composed of sodium soap. The interlocking mesh of said fibers and/or platelets imparts strength to the three-dimensional structure, even in the presence of relatively high levels of water or other soft materials; even when allowed to soak overnight in water.

The strength of the skeleton structure can be measured indirectly by the hardness of the shaped solid, as determined by the resistance to penetration of the solid using a Standard Weighted Penetrometer Probe. See Bar Hardness Test below for more details. The skeleton structure is of sufficient rigidity that a 25 mm thick or greater cleansing bar sample has a penetration of from zero mm to 12 mm, preferably from 1 mm to 10 mm, more preferably from 3 mm to 8 mm.

The present bars are distinguished from conventional transparent bars based on crystal size, as well as other characteristics. The crystals or crystal bundles that make-up the interlocking mesh structure of the present invention are of a size that diffracts light and consequently are greater than 400 nm in either diameter or length. On the other hand, conventional transparent bars gain their transparency by having crystal diameters or length less than the wavelength of white light, which is greater than about 400 nm and consequently do not diffract light.

Once formed, a bar (shaped solid) comprising the rigid skeletal structure of the present invention loses its rigidity when subjected to fracturing mechanical forces, e.g., those used in a conventional plodded bar making process as disclosed in US-A-4,812,253, Small et al., or US-A-4,820,447, Medcalf et al. This is because the fracturing mechanical forces, shear and break up the rigid, skeletal structure into smaller pieces. Thus, when a bar of the present invention is sheared in a plodder, a much softer bar results.

On the other hand, when a finished conventional bar is plodded or replodded the replodded conventional bar is still very hard. See Example 28 and Table 12 for more details on this point.

The skeletal structure contains substantial "void" areas which are filled by soft and/or liquid aqueous phases. It is a surprising aspect of this invention that the physical properties of the bar, such as bar hardness and little smear, are mostly dependent on the crystalline interlocking mesh structure, even when the other phases make up a majority of the materials present. In conventional bars, many components can impact the overall bar physical properties because the components either modify the phase and structure of the soap or synthetic surfactant components that primarily determine the bar's physical properties. The combination of two or more phases (e.g., soap and aqueous solution) drastically changes the colloidal structure, and consequently, the physical properties of a conventional bar.

Thus, conventional bars are more limited in the type, levels and composition of soft phase materials that can be incorporated into the bar than the present invention. Such phases include most materials that are either flowable liquids or materials that are softer than the minimum hardness of an acceptable bar. These phases include aqueous solutions, liquid crystalline phases composed of water and surfactant, polymers; particularly surfactant-containing crystalline phases, and especially hygroscopic surfactants, which tend to become soft and sticky when mixed with water or other liquid phases including water-soluble organics (e.g., propylene glycol and glycerine), hydrophobic materials (e.g., mineral oil, liquid triglycerides), or soft hydrophobic materials, e.g., petrolatum, low melting paraffin, and low melting triglycerides.

In physical terms, all these phases can be characterized as being flowable liquids or so soft that a Standard Weighted Penetrometer Probe, as defined herein, will penetrate all the way through a 12 mm thick sample. These phases can be selectively included in the structure of the present invention without loss of the interlocking mesh structure and certain desirable physical properties.

The invention is a non-transparent cleansing bar comprising at least two phases: (1) an aqueous phase having a penetration value of 12 mm for a 12 mm deep sample; said aqueous phase being soft or flowable at 25°C; (2) a rigid crystalline phase comprising a rigid crystalline phase skeleton structure comprising an interlocking, open three-dimensional mesh of neutralized mono- and/or di-carboxylic acid elongated crystals light diffracting having a diameter or length greater than 400 nm; wherein said cleansing bar comprising said rigid crystalline phase skeleton structure and said aqueous phase has a penetration value of of from zero to 12 mm for a 25 mm deep sample; and wherein said penetration values are measured as 25°C using a 247 gram Standard Weighted Penetrometer Probe having a conical needle attach to a 9 inch (22.9 cm) shaft weighing 47 grams, with 200 grams on top of said shaft for a total of said 247 grams, said conical needle having a 19/32 inch (1.51 cm) top and a 1/32 inch (0.08 cm) point.

In the above cleansing bar, said neutralized carboxylic acid is selected from the group consisting of: lithium and/or sodium neutralized: monocarboxylic acid (soap) and/or dicarboxylic acid; and mixtures thereof; wherein said monocarboxylic acid has a fatty alkyl(ene) chain of from about 12 to about 24 carbon atoms; wherein said dicarboxylic acid has a fatty alkyl(ene) chain of from about 12 to about 18 carbon atoms; and wherein at least about 80% of said carboxylic acid has saturated alkyl(ene) chains; and wherein said rigid crystalline phase skeleton structure occupies from above 3% to 75% of said cleansing bar by volume; and wherein said neutralized carboxylic acid comprises from above 5% to 75%; and wherein said cleansing bar contains from 15% to less than 94% water by weight of said cleansing bar.

The above cleansing bar is preferred when at least 80%, preferably 90%, of the carboxylic acid has the following general formula:
wherein:$\text{a + b = 8 to 20}$ each a, b = 0 to 20
X = H, OR,
R, or mixtures thereof
R = C₁-C₃ alkyl, H, or mixtures thereof
M = Na, Li, or mixtures thereof.

The above cleansing bar is more preferred when said $\text{a + b = 10-16}$ ; each of said a, b = 0-16; said X = H, OR; R = H; and M = Na.

The above cleansing bar is highly preferred when said elongated crystals are composed of fiber-like sodium fatty acid soap of which at least 25% of said saturated fatty alkyl chains is of a single chain length; and wherein said bar contains: from 15% to 75% by weight of said sodium soap; wherein the ratio of said unneutralized (free) carboxylic acid to soap is from 1:2 to 0. In other words, the free fatty acid is no more than 50% by weight of the soap in the formulation.

The above cleansing bar is preferred when said bar contains said sodium soap and water; and from 2% to 60% by weight of a synthetic surfactant selected from the group consisting of: alkyl sulfates, paraffin sulfonates, alkylglycerylether sulfonates, acyl sarcosinates, methylacyl taurates, linear alkyl benzene sulfonates, N-acyl glutamates, alkyl glucosides, alpha sulfo fatty acid esters, acyl isethionates, alkyl sulfosuccinates, alkyl ether carboxylates, alkyl phosphate esters, ethoxylated alkyl phosphate esters, methyl glucose esters, protein condensates, alkyl amine oxides, alkyl betaines, alkyl sultaines, the alkyl ether sulfates with 1 to 12 ethoxy groups, and mixtures thereof, wherein said surfactants contain C₈-C₂₂ alkyl chains.

The above cleansing bar is preferred when said synthetic surfactant is hygroscopic; said hygroscopic surfactant being defined as a surfactant which absorbs at least 20% of its dry weight in water at 26°C and 80% Relative Humidity in three days and wherein said bar is relatively non-swelling.

The above cleansing bar is preferred when said hygroscopic surfactant is selected from the group consisting of alpha sulfo fatty acid esters; alkyl sulfates; alkyl ether carboxylates; alkyl betaines; alkyl sultaines; alkyl amine oxides; alkyl ether sulfates; and mixtures thereof.

The above cleansing bar is preferred when the ratio of said water to said soap is from 1:1 to 5:1; said water is present at a level of from 25% to 60% by weight; wherein said fatty alkyl chains are C₁₄ to C₂₂ and said soap level in said bar is from 15% to 35% by weight; wherein at least 85% of said alkyl chains are saturated; wherein the weight ratio of said unneutralized (free) carboxylic acid to said soap is from 1:4 to 0; and wherein said synthetic surfactant level is from 4% to 25% by weight of the bar and said surfactant is selected from the group consisting of: sodium acyl isethionates, sodium acyl sarcosinates, sodium alpha sulfo fatty acid esters, sodium paraffin sulfonates, sodium alkyl ether sulfates, sodium alkyl sulfates, sodium linear alkyl benzene sulfonates, alkyl betaines, alkyl sultaines, and trialkyl amine oxides.

The above cleansing bar is preferred when the ratio of said water to soap ratio is from 1.5:1 to 2:1; the ratio of said unneutralized (free) carboxylic acid to said soap is from 1:6 to 0; said water level is from about 30% to about 45% by weight; said fatty alkyl chain is from C₁₄ to C₁₈; wherein at least 95% of said alkyl chains are saturated; said soap level is from 15% to 30% by weight; and said synthetic surfactant level is from 8% to 16% by weight.

The above cleansing bar is preferred when said bar contains from 0.1% to 40% by weight of a hydrophobic material selected from the group consisting of: microcrystalline wax, petrolatum, carnauba wax, palm wax, candelilla wax, sugarcane wax, vegetable derived triglycerides, beeswax, spemaceti, lanolin, wood wax, shellac wax, animal derived triglycerides, montar, ozokerite, ceresin, and Fischer-Tropsch wax.

The above cleansing bar is preferred when said bar contains from 2% to 35% by weight of said hydrophobic material selected from the group consisting of petrolatum and wax, said petrolatum and wax, and mixtures thereof melting melting 49°C (120°F) to 85°C (185°F).

The above cleansing bar is preferred when said bar comprises from 5% to 25% by weight of the bar of paraffin wax.

The above cleansing bar is preferred when said bar contains from 1% to 50% by weight of a non-volatile, water-soluble, nonionic organic material having a solubility of at least 5 parts in 10 parts of water; and wherein said water-soluble nonionic organic material is selected from the group consisting of a polyol of the structure:
where R₁ = H, C₁-C₄; R₂ = H, CH₃; and n = 1-200;
C₂-C₁₀ alkane diols; sorbitol; glycerine; sugars; sugar derivatives; urea; and
ethanol amines of the general structure (HOCH₂CH₂)ₓNH_{y} where x = 1-3; y = 0-2; and x+y = 3, and mixtures thereof.

The above cleansing bar is preferred when said bar contains from 2% to 40% by weight of said non-volatile, water-soluble, nonionic organic material.

The above cleansing bar is preferred when said non-volatile, water-soluble, nonionic organic material comprises from 5% to 20% by weight of the bar; and wherein said organic material is selected from the group consisting of: propylene glycol, glycerine, sucrose, and urea, and mixtures thereof.

The above cleansing bar is preferred when said bar contains said sodium soap, said water, and said synthetic surfactant, and from 0.1% to 70% by weight of other ingredients selected from the group consisting of:
from 1% to 10% by weight said potassium soap;
from 1% to 35% by weight said magnesium soap;
from 1% to 35% by weight said calcium soap;
from 1% to 15% by weight triethanolammonium soap;
from 1% to 60% by weight of impalpable water-insoluble materials selected from the group consisting of calcium carbonate and talc;
from 0.1% to 20% by weight of a polymeric skin feel aid; wherein said polymeric skin feel aid is selected from the group consisting of cationic polysaccharides, preferably cationic guar gum with molecular weights of 1,000 to 3,000,000; cationic polyalkylene imines, ethoxypolyalkylene imines, and poly[N-[-3-(dimethylammonio)propyl]-N'-[3-ethyleneoxyethylene dimethylammonio)propyl]urea dichloride]; silicone gum; and silicone fluids; JR polymers (RTM); Celequat (RTM);
from 0.5% to 25% by weight of aluminosilicate clay and/or other clays; wherein said aluminosilicates and clays are selected from the group consisting of zeolites; kaolin, kaolinite, montmorillonite, attapulgite, illite, bentonite, halloysite, and calcined clays;
from 1% to 50% by weight of salt and salt hydrates; and mixtures thereof; and wherein said salt and salt hydrate have a cation selected from the group consisting of: sodium, potassium, magnesium, calcium, aluminum, lithium, ammonium, monoethanol ammonium, diethanolammonium, and triethanolammonium; and wherein said salt and salt hydrate have an anion selected from the group consisting of: chloride, bromide, sulfate, metasilicate, orthophosphate, pyrophosphate, polyphosphate, metaborate, tetraborate, carbonate, bicarbonate, hydrogen phosphate, methyl sulfate, and mono- and polycarboxylate of 6 carbon atoms or less.

The above cleansing bar is preferred when said elongated crystals contain platelets and wherein said soap consists of lithium neutralized monocarboxylic acid.

The above cleansing bar is preferred when said elongated crystals are fiber-like and wherein said neutralized dicarboxylic acid is the disodium salt 1,12-dodecanedioic acid and wherein said neutralized dicarboxylic acid comprises from 20% to 70% by weight of said bar.

A process of making the above cleansing bar of the present invention comprises the steps of:
I. forming an aqueous molten liquid comprising 15% to 94% water and from 6% to 75% by weight said neutralized carboxylic acid;
II. pouring said molten liquid into a bar shaped mold; and
III. crystallizing said molded molten liquid by cooling to provide said cleansing bar,
wherein the aqueous molten liquid is made by neutralizing an aqueous mixture of said carboxylic acid with sodium hydroxide or lithium hydroxide with stirring at a temperature of from about 50°C (120°F) to about 95°C (205°F) and wherein from 2% to 15% by weight of said bar is a "crystallization enhancing salt" selected from the group consisting of: sodium or lithium salt of sulfate, chloride, acetate and citrate, and mixtures thereof and wherein when said aqueous molten liquid aqueous phase contains from 2% to 40% by weight of a solubilizing aid selected from the group consisting of:
(a) non-volatile, water-soluble nonionic organic solvents selected from the group consisting of: a polyol of the structure: where R₁ = H, C₁-C₄; R₂ = H, CH₃; and n = 1-200; C₂-C₁₀ alkane diols; sorbitol; glycerine; sugars; sugar derivatives; urea; and ethanol amines of the general structure (HOCH₂CH₂)ₓNH_{y} where x = 1-3; y = 0-2; and x+y = 3;
(b) alcohols of from 1 to 5 carbon atoms;
(c) synthetic surfactant selected from the group consisting of: alkyl sulfates, paraffin sulfonates, alkyl glyceryl ether sulfonates, anionic acyl sarcosinates, methyl acyl taurates, linear alkyl benzene sulfonates, N-acyl glutamates, alkyl glucosides, alpha sulfo fatty acid esters, acyl isethionates, alkyl sulfosuccinates, alkyl ether carboxylates, alkyl phosphate esters, ethoxylated alkyl phosphate esters, methyl glucose esters, protein condensates, alkyl amine oxides, alkyl betaines, alkyl sultaines, the alkyl ether sulfates with 1 to 12 ethoxy groups, and mixtures thereof, wherein said surfactants contain C₈-C₂₂ alkylene chains; and
   mixtures thereof; and
wherein said solubilizing aid is added to increase the level of said neutralized carboxylic acid dissolved in said continuous molten aqueous phase in step I.

The above process is preferred when said aqueous phase contains from 20% to 100% water by weight of said aqueous phase.

The above process is preferred when said rigid crystalline phase contains from 75% to 100% of said neutralized carboxylic acid by weight of said crystalline phase.

The above process is preferred when said bar has a penetration value of from 3 mm to 9 mm for said 25 mm bar sample.

The above process is preferred when said bar has miscellaneous non-carboxylic acid phases comprising droplets or crystals selected from waxes, petrolatum, clays, and the like.

A preferred embodiment of the present invention is: a personal cleansing bar composition comprising a rigid, crystalline interlocking mesh of elongated sodium soap crystals; said soap bar comprising: from 15% to 50% by weight sodium fatty acid soap composed of at least 50% saturated fatty alkylene chains having 12-24 carbon atoms of which at least 25% of said saturated fatty alkyl chains is of a single chain length; from 15% to 60% water by weight; and from 2% to 60% by weight of a hygroscopic synthetic surfactant wherein said hygroscopic synthetic surfactant is selected from surfactants which absorb at least 20% of their dry weight in water at 26°C and 80% Relative Humidity in three days.

The above preferred personal cleansing bar is more preferred when said hygroscopic synthetic surfactant is selected from the group consisting of alpha sulfo fatty acid esters; alkyl sulfates; alkyl ether carboxylates; alkyl betaines; alkyl sultaines; alkyl amine oxides; alkyl ether sulfates; and mixtures thereof.

This preferred personal cleansing bar is more preferred when said bar contains from 0.5% to 40% by weight of salts and/or salt hydrates selected from the group consisting of: sodium chloride, sodium sulfate, disodium hydrogen phosphate, sodium pyrophosphate, sodium tetraborate, sodium acetate, sodium citrate, and other compatible salts of inorganic acids and short chain organic acids.

A highly preferred cleansing bar comprises: various combinations of the core structure of sodium soap fibers, water, mild synthetic surfactants, bar appearance stabilizers, skin mildness aides and other cleansing bar adjuvants. Such preferred bar can be formulated to have essentially no bar smear.

Some preferred bars of the present invention comprise: a rigid, interlocking mesh of neutralized carboxylic acid fiber-like core consisting essentially of sodium fatty acid soap composed of at least 50% saturated fatty alkyl chains having 12 to 24 carbon atoms. Preferably at least about 25% of said saturated alkyl chains are of a single chain length.

Some compositions of this invention comprise the above-defined rigid mesh with water and without water. These compositions must be formed with water or another suitable solvent system. The compositions can be made with large amounts of water and the water level in the final composition can be reduced to as low as 1% or 2% by weight.

However, it is a special advantage of some structures described herein that they can be dehydrated without loss of the integrity of the mesh. Some preferred shaped solids can be dehydrated without appreciable change in their outer dimensions. Other bars shrink while maintaining their three-dimensional form. Some bars herein have the unique characteristic that they are not destroyed by dehydration.

More complex bars of the present invention comprise a skeletal structure comprising other salts of fatty acids selected from potassium, magnesium, triethanolammonium and/or calcium soaps used in combination with the selected levels of sodium and/or lithium soaps. More complex cleansing bars can contain surprisingly large amounts of water, mild synthetic surfactants, bar appearance stabilizers, skin mildness aids and other cleansing bar adjuvants; yet are mild and have very good low smear.

Tables 1-3 set out some preferred bars which are made with the sodium salts of the fatty carboxylic acid (FA) soap.

The percentages, ratios, and parts herein are on a total composition weight basis, unless otherwise specified. All levels and ranges herein are approximations unless otherwise specified.

**TABLE 1**

| Preferred Bars, Chain Lengths and Levels | | | |
|---|---|---|---|
| | Preferred | More Preferred | Most Preferred |
| Water Level | 15-94% | 25-60% | 30-45% |
| Water:Soap Ratio | 0.7:1 | 1:1-5:1 | 1.5:1-2:1 |
| FA Chain Length | C₁₂₋₂₄ | C₁₄₋₂₂ | C₁₄₋₁₈ |
| FA Soap Level in Total Formulation | 6-50% | 15-35% | 15-30% |

All highs and lows are not necessarily shown in Table 1. For example, some selected sodium soap can be used at a level up to 75% by weight. Thus, the range is from 5% to 75% by weight. The preferred levels and ratios can vary from cation to cation, etc., and from mono- to polycarboxylic acids.

The bars shown in Table 1 are made with the level of water indicated, but the water level of the final bars can be reduced to provide bars which contain reduced levels of water or even little or no water. A preferred level of water is from 20% to 80% by weight of the bar.

Table 2 below shows some preferred levels of soaps of a single FA chain length. Table 3 shows some preferred levels of unsaturation in the FA's used in the compositions of the present invention. Some preferred compositions contain little or no short chain FA's of ten carbon atoms or less. The terms "soap", "fatty acid (FA) salts" and "monocarboxylic acid salts" as used herein are sometimes interchangeable. "Soap" is used since it is easier to relate to and is the preferred embodiment.

**TABLE 2**

| The % Soap of Single Chain Length (of Total Fibrous Soap Content) | | | |
|---|---|---|---|
| | Preferred | More Preferred | Most Preferred |
| C₁₂₋₂₄ | 25-100% | 50-100% | 75-100% |

**TABLE 3**

| The Total % Unsaturated or Low (C₁₀ or less) Chain Length Soaps | | | |
|---|---|---|---|
| | Broad | Preferred | More Preferred |
| C₁₂ | 0-15% | 0-5% | 0-1% |
| C₁₄₋₂₄ | 0-50% | 0-10% | 0-1% |

The highs and lows of some key preferred optional ingredients for complex soap bar compositions of this invention are set out in Table 4. None of these ingredients is essential for the basic, preferred bar core structure. Zero is the lowest level for each optional ingredient. Some preferred bars can contain a total of from 0.1% up to 70% by weight of such ingredients. The idea here is that the core bars can contain large amounts of other ingredients besides soap and water. The levels set out in Table 4 are particularly illustrative for bars containing from more than 5% to 75% by weight selected sodium soap and other ingredients.

It should be understood that solid shapes can be made with just lithium soap or just neutralized polycarboxylic acid, but would be expected to be somewhat different from the levels and ratios given for sodium soaps.

**TABLE 4**

| Highs and Lows Wt.% of Other Ingredients for More Complex Sodium Soap Bars | | | |
|---|---|---|---|
| | Preferred | More Preferred | Most Preferred |
| Neutralized Dicarboxylic Acid | 1-40% | 2-30% | 5-25% |
| Lithium "Soap" | 1-40% | 2-30% | 5-25% |
| Potassium Soap | 1-10% | 2-10% | 5-8% |
| Magnesium or Calcium Soap | 1-35% | 1-12% | 3-8% |
| Triethanolammonium Soap | 1-15% | 2-15% | 5-10% |
| Synthetic Surfactant | 1-60% | 4-25% | 8-16% |
| Other Salts and Salt Hydrates | 0.5-50% | 1-25% | 2-15% |
| Non-Volatile, Water-Soluble Nonionic Organics | 1.0-50% | 2-40% | 5-20% |
| Polymeric Mildness Enhancers | 0.1-20% | 0.25-10% | 1-5% |
| Waxes | 0.1-40% | 2-35% | 3-10% |
| Other Impalpable Water-insolubles | 1-60% | 4-25% | 8-16% |
| Aluminosilicates/Clay | 0.5-25% | 1-10% | 3-8% |

The soaps useful in the present invention can be of the same alkyl chain lengths, i.e., which are selected from the 12 to 24 carbon atoms as set out in Table 2. The same chain lengths apply for the other non-sodium soaps used in the bars of the present invention.

The sodium soap is preferably at least 50% by weight of the soap present in the bar.

The levels of potassium soap and/or triethanolammonium soap should not exceed one-half, preferably one-third, more preferably less than one-fourth, that of the sodium soap and the level of magnesium soap should not exceed about one-third of the level of sodium soap, and is preferably less than about one-fourth that of the sodium soap.

The total of other soaps, save lithium soap, should preferably not exceed one-half, preferably one-third, of the sodium soap.

The synthetic detergent constituent of the bar compositions of the invention can be designated as being a detergent from the class consisting of anionic, nonionic, amphoteric and zwitterionic synthetic detergents. Both low and high lathering and high and low water-soluble surfactants can be used in the bar compositions of the present invention.

Examples of suitable synthetic detergents for use herein are these described in US-A-3,351,558, Zimmerer, issued Nov. 7, 1967, at column 6, line 70 to column 7, line 74.

Examples include the water-soluble salts of organic, sulfonic acids and of aliphatic sulfuric acid esters, that is, water-soluble salts of organic sulfuric reaction products having in the molecular structure an alkyl radical of from 10 to 22 carbon atoms and a radical selected from the group consisting of sulfonic acid and sulfuric acid ester radicals.

Synthetic sulfate detergents of special interest are the normally solid alkali metal salts of sulfuric acid esters of normal primary aliphatic alcohols having from 10 to 22 carbon atoms. Thus, the sodium and potassium salts of alkyl sulfuric acids obtained from the mixed higher alcohols derived by the reduction of tallow or by the reduction of coconut oil, palm oil, stearine, palm kernel oil, babassu kernel oil or other oils of the coconut group can be used herein.

Other aliphatic sulfuric acid esters which can be suitably employed include the water-soluble salts of sulfuric acid esters of polyhydric alcohols incompletely esterified with high molecular weight soap-forming carboxylic acids. Such synthetic detergents include the water-soluble alkali metal salts of sulfuric acid esters of higher molecular weight fatty acid monoglycerides such as the sodium and potassium salts of the coconut oil fatty acid monoester of 1,2-hydroxypropane-3-sulfuric acid ester, sodium and potassium monomyristoyl ethylene glycol sulfate, and sodium and potassium monolauroyl diglycerol sulfate.

The synthetic surfactants and other optional materials useful in conventional cleaning products are also useful in the present invention. In fact, some ingredients such as certain hygroscopic synthetic surfactants which are normally used in liquids and which are very difficult to incorporate into normal cleansing bars are very compatible in the bars of the present invention. Thus, essentially all of the known synthetic surfactants which are useful in cleansing products are useful in the compositions of the present invention. The cleansing product patent literature is full of synthetic surfactant disclosures. Some preferred surfactants as well as other cleansing product ingredients are disclosed in the following references:

| Pat. No. | Issue Date | Inventor(s) |
|---|---|---|
| US-A-4,061,602 | 12/1977 | Oberstar et al. |
| US-A-4,234,464 | 11/1980 | Morshauser |
| US-A-4,472,297 | 9/1984 | Bolich et al. |
| US-A-4,491,539 | 1/1985 | Hoskins et al. |
| US-A-4,540,507 | 9/1985 | Grollier |
| US-A-4,565,647 | 1/1986 | Llenado |
| US-A-4,673,525 | 6/1987 | Small et al. |
| US-A-4,704,224 | 11/1987 | Saud |
| US-A-4,788,006 | 11/1988 | Bolich, Jr., et al. |
| US-A-4,812,253 | 3/1989 | Small et al. |
| US-A-4,820,447 | 4/1989 | Medcalf et al. |
| US-A-4,906,459 | 3/1990 | Cobb et al. |
| US-A-4,923,635 | 5/1990 | Simion et al. |
| US-A-4,954,282 | 9/1990 | Rys et al. |

Some preferred synthetic surfactants are shown the Examples herein. Preferred synthetic surfactant systems are selectively designed for bar appearance stability, lather, cleansing and mildness.

It is noted that surfactant mildness can be measured by a skin barrier destruction test which is used to assess the irritancy potential of surfactants. In this, test the milder the surfactant, the lesser the skin barrier is destroyed. Skin barrier destruction is measured by the relative amount of radio-labeled water (³H-H₂O) which passes from the test solution through the skin epidermis into the physiological buffer contained in the diffusate chamber. This test is described by T.J. Franz in the J. Invest. Dermatol., 1975, 64, pp. 190-195; and in US-A-4,673,525, Small et al., issued June 16, 1987, and which disclose a mild alkyl glyceryl ether sulfonate (AGS) surfactant based synbar comprising a "standard" alkyl glyceryl ether sulfonate mixture. Barrier destruction testing is used to select mild surfactants. Some preferred mild synthetic surfactants are disclosed in the above Small et al. patents and Rys et al. Some specific examples of preferred surfactants are used in the Examples herein.

Some examples of good lather enhancing detergent surfactants, mild ones, are e.g., sodium lauroyl sarcosinate, alkyl glyceryl ether sulfonate, sulfonated fatty esters, paraffin sulfonates, and sulfonated fatty acids.

Numerous examples of other surfactants are disclosed in the patents referred to herein. They include other alkyl sulfates, anionic acyl sarcosinates, methyl acyl taurates, N-acyl glutamates, acyl isethionates, alkyl sulfosuccinates, alkyl phosphate esters, ethoxylated alkyl phosphate esters, trideceth sulfates, protein condensates, mixtures of ethoxylated alkyl sulfates and alkyl amine oxides, betaines, sultaines, and mixtures thereof. Included in the surfactants are the alkyl ether sulfates with 1 to 12 ethoxy groups, especially ammonium and sodium lauryl ether sulfates.

Alkyl chains for these other surfactants are C₈-C₂₂, preferably C₁₀-C₁₈. Alkyl glycosides and methyl glucose esters are preferred mild nonionics which may be mixed with other mild anionic or amphoteric surfactants in the compositions of this invention. Alkyl polyglycoside detergents are useful lather enhancers. The alkyl group can vary from 8 to 22 and the glycoside units per molecule can vary from 1.1 to 5 to provide an appropriate balance between the hydrophilic and hydrophobic portions of the molecule. Combinations of C₈-C₁₈, preferably C₁₂-C₁₆, alkyl polyglycosides with average degrees of glycosidation ranging from 1.1 to 2.7, preferably from 1.2 to 2.5, are preferred.

Sulfonated esters of fatty esters are preferred wherein the chain length of the carboxylic acid is C₈-C₂₂, preferably C₁₂-C₁₈; the chain length of the ester alcohol is C₁-C₆. These include sodium alpha sulfomethyl laurate, sodium alpha sulfomethyl cocoate, and sodium alpha sulfomethyl tallowate.

Amine oxide detergents are good lather enhancers. Some preferred amine oxides are C₈-C₁₈, preferably C₁₀-C₁₆, alkyl dimethyl amine oxides and C₈-C₁₈, preferably C₁₂-C₁₆, fatty acyl amidopropyl dimethyl amine oxides and mixtures thereof.

Fatty acid alkanolamides are good lather enhancers. Some preferred alkanolamides are C₈-C₁₈, preferably C₁₂-C₁₆, monoethanolamides, diethanolamides, and monoisopropanolamides and mixtures thereof.

Other detergent surfactants are alkyl ethoxy carboxylates having the general formula

RO(CH₂CH₂O)ₖCH₂COO⁻M⁺

wherein R is a C₈₋₂₂ alkyl group, k is an integer ranging from 0 to 10, and M is a cation; and polyhydroxy fatty acid amides having the general formula
wherein R¹ is H, a C₁₋₄ alkyl group, 2-hydroxy ethyl, 2-hydroxy propyl, or mixtures thereof, R² is a C₅₋₃₁ hydrocarbyl, and Z is a polyhydroxyhydrocarbyl having a linear hydrocarbyl chain with at least 3 hydroxyl groups directly connected to the chain, or an alkoxylated derivative thereof.

Betaines are good lather enhancers. Betaines such as C₈-C₁₈, preferably C₁₂-C₁₆, alkyl betaines, e.g., coco betaines or C₈-C₁₈, preferably C₁₂-C₁₆, acyl amido betaines, e.g., cocoamidopropyl betaine, and mixtures thereof, are preferred.

Some of the preferred surfactants are hygroscopic synthetic surfactants which absorb at least 20% of their dry weight at 26°C and 80% relative humidity in three days. Hygroscopic surfactants help to improve bar lather. Some preferred hygroscopic synthetic surfactants are listed below. Note that all are not hygroscopic.

### Hygroscopicity of Some Surfactants

The hygroscopic surfactants are defined herein as having a minimum of 20% total moisture gain after 3 days at 26°C and 80% Relative Humidity.

### Class: Nonionic

| Sulfonates | Total % Moisture Pick-Up* |
|---|---|
| Sodium C₈ Glyceryl Ether Sulfonate | 39.8 |
| Sodium C₁₂₋₁₄ Glyceryl Ether Sulfonate | 22.9 |
| Sodium C₁₆ Glyceryl Ether Sulfonate | 71.4 |
| Sodium Cocomonoglyceride Sulfonate | 3.5 |

| | |
|---|---|
| *3 days, 26°C/80% Relative Humidity | |

Sodium Salt of C₈₋₁₆ Alkyl Glyceryl Ether Sulfonates

| Alpha Sulfo Esters and Acids | Total % Moisture Pick-Up* |
|---|---|
| Sodium Alpha Sulfo Methyl Laurate/Myristate | 39.3 |
| Sodium Alpha Sulfo Methyl Myristate | 44.5 |
| Sodium Alpha Sulfo Hexyl Laurate | 23.2 |
| Sodium Alpha Sulfo Methyl/Hexyl Laurate and Myristate | 26.3 |
| Sodium Alpha Sulfo Methyl Palmitate | 3.7 |
| Sodium Alpha Sulfo Methyl Stearate | 4.2 |
| Sodium 2-Sulfo Lauric Acid | 0.2 |
| Sodium 2-Sulfo Palmitic Acid | 3.8 |
| Sodium 2-Sulfo Stearic Acid | 0.0 |
| Na+R₁-C(SO₃⁻)-CO₂R₂ R₁ = C₈₋₁₄ alkyl; R₂ = C₁₋₈ alkyl | |

| | |
|---|---|
| *3 days, 26°C/80% Relative Humidity | |

| Sodium Alkyl Isethionates | Total % Moisture Pick-Up* |
|---|---|
| Sodium Lauryl Isethionate | 31.7 |
| Sodium Cocoyl Isethionate | 11.0 |

| | |
|---|---|
| *3 days, 26°C/80% Relative Humidity | |

| Sarcosinates | Total % Moisture Pick-Up* |
|---|---|
| Sodium Lauryl Sarcosinate | 8.8 |
| Sodium Stearyl Sarcosinate | 13.3 |
| Sodium Cocoyl Sarcosinate | 18.7 |

| | |
|---|---|
| *3 days, 26°C/80% Relative Humidity | |

| Alkyl Sulfates | Total % Moisture Pick-Up* |
|---|---|
| Sodium Lauryl Sulfate | 28.2 |
| Sodium Laureth-1 Sulfate | 37.6 |
| Sodium Oleyl Sulfate | 20.3 |
| Sodium Cetearyl Sulfate | 4.7 |
| Sodium Cetyl Sulfate | 2.25 |
| Na+R₁(OCH₂CH₂)ₙOSO₃⁻ R₁ = C₈₋₁₄ alkyl, C₁₆₋₂₀ alkyl(ene) with at least one double bond, n = 0-18 | |

| | |
|---|---|
| *3 days, 26°C/80% Relative Humidity | |

| Acyl Glutamates | Total % Moisture Pick-Up* |
|---|---|
| Sodium Cocoyl Glutamate | 26.7 |
| Sodium Lauryl Glutamate | 17.8 |
| Sodium Myristyl Glutamate | 18.1 |
| Sodium Stearyl Glutamate | 12.0 |

| | |
|---|---|
| *3 days, 26°C/80% Relative Humidity | |

| Alkyl Ether Carboxylates | Total % Moisture Pick-Up* |
|---|---|
| Sodium Laureth-5 Carboxylate | 32.2 |
| Sodium Palmityl-20 Carboxylate | 50.2 |
| Na+R₁-(O-CH₂CH₂)ₙCO₂⁻ R₁ = C₈₋₁₈ alkyl, n = 1-30 | |

| | |
|---|---|
| *3 days, 26°C/80% Relative Humidity | |

| Sulfosuccinates | Total % Moisture Pick-Up* |
|---|---|
| Disodium Laureth Sulfosuccinate | 33.6 |

| | |
|---|---|
| *3 days, 26°C/80% Relative Humidity | |

| Phosphates | Total % Moisture Pick-Up* |
|---|---|
| Sodium Monoalkyl (70% C₁₂/30% C₁₄) Phosphate | 21.1 |

| | |
|---|---|
| *3 days, 26°C/80% Relative Humidity | |

### Class: Amphoterics

| Betaines | Total % Moisture Pick-Up* |
|---|---|
| Coco Betaine | 70.0 |
| Cocoamidopropyl Betaine | 48.2 |
| Palmitylamidopropyl Betaine | 46.5 |
| Isostearamidopropyl Betaine | 44.3 |

| | |
|---|---|
| *3 days, 26°C/80% Relative Humidity | |

| Sultaines | Total % Moisture Pick-Up* |
|---|---|
| Cocoamidopropylhydroxy Sultaine | 59.5 |

| | |
|---|---|
| *3 days, 26°C/80% Relative Humidity | |

| Amine Oxides | Total % Moisture Pick-Up* |
|---|---|
| Palmityl Dimethyl Amine Oxide | 34.0 |
| Myristyl Dimethyl Amine Oxide | 46.0 |
| Cocoamidopropyl Amine Oxide | 43.3 |

| | |
|---|---|
| *3 days, 26°C/80% Relative Humidity | |

| Protein Derived | Total % Moisture Pick-Up* |
|---|---|
| Na/TEA C₁₂ Hydrolyzed Keratin | 34.7 |

| | |
|---|---|
| *3 days, 26°C/80% Relative Humidity | |

Polymeric skin mildness aids are disclosed in the Small et al. and Medcalf et al. patents. Both cationic polysaccharides and cationic synthetic polymers are disclosed. The cationic synthetic polymers useful in the present invention are cationic polyalkylene imines, ethoxypolyalklene imines, and poly[N-[-3-(dimethylammonio)-propyl]-N'-[3-(ethyleneoxyethylene dimethylammonio)propyl]urea dichloride] the latter of which is available from Miranol Chemical Company, Inc. under the trademark of Miranol (RTM) A-15, CAS Reg. No. 68555-36-2.

Preferred cationic polymeric skin conditioning agents of the present invention are those cationic polysaccharides of the cationic guar gum class with molecular weights of 1,000 to 3,000,000. More preferred molecular weights are from 2,500 to 350,000. These polymers have a polysaccharide backbone comprised of galactomannan units and a degree of cationic substitution ranging from about 0.04 per anhydroglucose unit to about 0.80 per anhydroglucose unit with the substituent cationic group being the adduct of 2,3-epoxypropyltrimethyl ammonium chloride to the natural polysaccharide backbone. Examples are JAGUAR C-14-S (RTM), C-15 (RTM) and C-17 (RTM) sold by Celanese Corporation. In order to achieve the benefits described in this invention, the polymer must have characteristics, either structural or physical which allow it to be suitably and fully hydrated and subsequently well incorporated into the soap matrix.

A mild skin cleansing bar of the present invention can contain from 0.5% to 20% by weight of a mixture of a silicone gum and a silicone fluid wherein the gum:fluid ratio is from 10:1 to 1:10, preferably from 4:1 to 1:4, most preferably from 3:2 to 2:3.

Silicone gum and fluid blends have been disclosed for use in shampoos and/or conditioners in US-A-4,906,459, Cobb et al., issued March 6, 1990; US-A-4,788,006, Bolich, Jr. et al., issued Nov. 29, 1988; US-A-4,741,855, Grote et al., issued May 3, 1988; US-A-4,728,457, Fieler et al., issued March 1, 1988; US-A-4,704,272, Oh et al., issued Nov. 3, 1987; and US-A-2,826,551, Geen, issued March 11, 1958.

The silicone component can be present in the bar at a level which is effective to deliver a skin mildness benefit, for example, from 0.5% to 20% by weight, preferably from 1.5% to 16% by weight, and most preferably from 3% to 12% by weight of the composition. Silicone fluid, as used herein, denotes a silicone with viscosities ranging from 5 to 600,000 mm²s⁻¹ (centistokes), most preferably from 350 to 100,000 mm²s⁻¹ (centistokes), at 25°C. Silicone gum, as used herein, denotes a silicone with a mass molecular weight of from 200,000 to 1,000,000 and with a viscosity of greater than 600,000 mm²s⁻¹ (centistokes). The molecular weight and viscosity of the particular selected siloxanes will determine whether it is a gum or a fluid. The silicone gum and fluid are mixed together and incorporated into the compositions of the present invention.

Other ingredients of the present invention are selected for the various applications. E.g., perfumes can be used in formulating the skin cleansing products, generally at a level of from 0.1% to 2.0% by weight of the composition. Alcohols, hydrotropes, colorants, and fillers such as talc, clay, water-insoluble, impalpable calcium carbonate and dextrin can also be used. Cetearyl alcohol is a mixture of cetyl and stearyl alcohols. Preservatives, e.g., sodium ethylenediaminetetraacetate (EDTA), generally at a level of less than 1% by weight of the composition, can be incorporated in the cleansing products to prevent color and odor degradation. Antibacterials can also be incorporated, usually at levels up to 1.5% by weight. The above patents disclose or refer to such ingredients and formulations which can be used in the bars of this invention.

Some bars of this invention contain from about more than 5% to 75% by weight said sodium fatty acid soap fibers; from 10% to less than 94% by weight water; and at least 1% by weight of another bar ingredient selected from: other soaps, moisturizers, colorants, solvents, fillers, synthetic detergent surfactants, polymeric skin feel and mildness aids, perfumes, preservatives, and mixtures thereof.

Some bars of this invention comprise: more 5% to 50% by weight fibrous sodium fatty acid soap composed of at least 50% saturated fatty alkyl chains having 12-24 carbon atoms of which at least 25% of said saturated fatty alkyl chains is of a single chain length.

Some bars of this invention comprise said fibers which occupy from 3% to 75% by weight, preferably from 15% to 40% by weight, of the volume of the bar structure.

Some bars comprise a rigid, low smearing structure of: more than 5% to 75% by weight sodium fatty acid soap composed of at least 50% saturated fatty alkyl chains having 12-24 carbon atoms of which at least 25% of said saturated fatty alkyl chains is of a single chain length; from 10% to 94% by weight water; and 0% to a total of 70% by weight of other selected soap bar ingredients selected from the group set out above in Table 4.

Some personal cleansing soap bar compositions comprise a rigid interlocked mesh of sodium soap fibers; wherein the sodium fatty acid soap is composed of at least 50% by weight saturated fatty alkyl chains having 12-24 carbon atoms of which at least about 25% of said saturated fatty alkyl chains is of a single chain length; and from 2% to 40% by weight of a hygroscopic synthetic surfactant wherein said hygroscopic synthetic surfactant is selected from surfactants which absorb at least 20% of its dry weight in water at 26°C and 80% Relative Humidity in three days.

Bar appearance (water-retaining and/or shrinkage prevention) aids are preferably selected from the group consisting of:
compatible salt and salt hydrates;
water-soluble organics such as polyols, urea;
aluminumosilicates and clays; and
mixtures thereof, as set out above in Table 4.

Water-soluble organics are also used to stabilize the appearance of the bar soaps of the present invention. Some preferred water-soluble organics are propylene glycol, glycerine, ethylene glycol, sucrose, and urea, and other compatible polyols.

A particularly suitable water-soluble organic is propylene glycol. Other compatible organics include polyols, such as ethylene glycol or 1,7-heptane-diol, respectively the mono- and polyethylene and propylene glycols of up to about 8,000 molecular weight, any mono-C₁₋₄ alkyl ethers thereof, sorbitol, glycerol, glycose, diglycerol, sucrose, lactose, dextrose, 2-pentanol, 1-butanol, mono- di- and triethanolammonium, 2-amino-1-butanol, and the like, especially the polyhydric alcohols.

The term "polyol" as used herein includes non-reducing sugar, e.g., sucrose. Sucrose will not reduce Fehling's solution and therefore is classified as a "non-reducing" disaccharide. Unless otherwise specified, the term "sucrose" as used herein includes sucrose, its derivatives, and similar non-reducing sugars and similar polyols which are substantially stable at a soap processing temperature of up to about 210°F (98°C), e.g., trialose, raffinose, and stachyose; and sorbitol, lactitol and maltitol.

Compatible salt and salt hydrates are used to stabilize the bar soap appearance via the retention of water. Some preferred salts are sodium chloride, sodium sulfate, disodium hydrogen phosphate, sodium pyrophosphate, sodium tetraborate.

Generally, compatible salts and salt hydrates include the sodium, potassium, magnesium, calcium, aluminum, lithium, and ammonium salts of inorganic acids and small (6 carbons or less) carboxylic or other organic acids, corresponding hydrates, and mixtures thereof, are applicable. The inorganic salts include chloride, bromide, sulfate, metasilicate, orthophosphate, pyrophosphate, polyphosphate, metaborate, tetraborate, and carbonate. The organic salts include acetate, formate, methyl sulfate, and citrate.

Water-soluble amine salts can also be used. Monoethanolamine, diethanolamine, and triethanolammonium (TEA) chloride salts are preferred.

Aluminosilicates and other clays are useful in the present invention. Some preferred clays are disclosed in US-A-4,605,509 and US-A-4,274,975.

Other types of clays include zeolite, kaolinite, montmorillonite, attapulgite, illite, bentonite, and halloysite. Another preferred clay is kaolin.

Waxes include petroleum based waxes (paraffin, microcrystalline, and petrolatum), vegetable based waxes (carnauba, palm wax, candelilla, sugarcane wax, and vegetable derived triglycerides) animal waxes (beeswax, spemaceti, wool wax, shellac wax, and animal derived triglycerides), mineral waxes (montar, ozokerite, and ceresin) and synthetic waxes (Fischer-Tropsch).

A preferred wax is used in the Examples herein. A useful wax has a melting point (M.P.) of from about 120°F to about 185°F (49°-85°C), preferably from about 125°F to about 175°F (52°-79°C). A preferred paraffin wax is a fully refined petroleum wax having a melting point ranging from about 130°F to about 140°F (49°-60°C). This wax is odorless and tasteless and meets FDA requirements for use as coatings for food and food packages. Such paraffins are readily available commercially. A very suitable paraffin can be obtained, for example from The Standard Oil Company of Ohio under the trade name Factowax R-133 (RTM).

Other suitable waxes are sold by the National Wax Co. under the trade names of 9182 (RTM) and 6971 (RTM), respectively, having melting points of 131°F and 130°F (-55°C).

The paraffin preferably is present in the bar in an amount ranging from 5% to 20% by weight. The paraffin ingredient is used in the product to impart skin mildness, plasticity, firmness, and processability. It also provides a glossy look and smooth feel to the bar.

The paraffin ingredient is optionally supplemented by a microcrystalline wax. A suitable microcrystalline wax has a melting point ranging, for example, from about 140°F (60°C) to about 185°F (85°C), preferably from about 145°F (62°C) to about 175°F (79°C). The wax preferably should meet the FDA requirements for food grade microcrystalline waxes. A very suitable microcrystalline wax is obtained from Witco Chemical Company under the trade name Multiwax X-145A (RTM). The microcrystalline wax preferably is present in the bar in an amount ranging from 0.5% to 5% by weight. The microcrystalline wax ingredient imparts pliability to the bar at room temperatures.

### EXAMPLES

The following examples are illustrative. Unneutralized or "free" fatty acids, as used in the examples, are of the same chain lengths as those used to make the soaps, unless otherwise specified. All levels and ranges, temperatures, results, etc., used herein, are approximations unless otherwise specified.

### A Frame Process for Making the Bars of the Present Invention

The cleansing bars in the Examples are made by the following procedure unless otherwise specified:
1. Fatty acid precursor, propylene glycol, sodium chloride, and water (excluding water coming in with other raw materials) are mixed and heated to 71°C.
2. Caustic solution (50% sodium hydroxide) is added and the mixture is stirred until smooth forming an aqueous molten liquid comprising from 15% to 94% by weight water and from 5.5% to 75% by weight soap (neutralized carboxylic acid). The temperature during neutralization of the molten liquid increases to ∼95°C.
3. Other ingredients are added preferably in the following order and the temperature is maintained at ∼88°C: coco betaine; sodium lauroyl sarcosinate; or sodium alpha-sulfo methyl cocoate: kaolin clay; or hydrated zeolite (synthetic sodium aluminosilicate); and paraffin. Perfume is added last.
4. The molten liquid mixture is poured into shaped molds.
5. The molten liquid crystallizes (solidifies) on cooling to room temperature and the resultant bars are removed from the moulds.

The bars of the examples are made using the above general procedure, unless otherwise specified.

It is important to note that, when the formulations which are used in the Examples of the present invention are subjected to a conventional plodding or freezer process very soft or no bars are formed. Example II is a very highly preferred overall bar.

**TABLE 5**

| Preferred Bars | | | | |
|---|---|---|---|---|
| Ingredient | Ex. I (Wt.%) | Ex. II (Wt.%) | Ex. III (Wt.%) | Ex. IV (Wt.%) |
| Na C₁₄ Soap | 20 | 20 | - | - |
| Na C₁₆ Soap | - | - | 20 | 16 |
| K C₁₆ Soap | - | - | - | 4 |
| Free Fatty Acid | 1 | 1 | 1 | 1 |
| Sodium Lauroyl Sarcosinate | 7 | 7 | 12 | - |
| Sodium Alpha Sulfo Methyl Cocoate | - | - | - | 7 |
| Coco Betaine | 5 | 5 | 7 | 5 |
| Sodium Chloride | 3.0 | 3.0 | 3.0 | 3.0 |
| Propylene Glycol | 14.5 | 14.5 | 14.5 | 15.0 |
| Hydrated Zeolite A (Aluminosilicate) | 4.0 | | 4.0 | - |
| Kaolin Clay | | 4.0 | - | 4.0 |
| Paraffin (M.P.=55°C) | 6.5 | 6.5 | 4.5 | - |
| Perfume | 1 | 1 | 1 | 1 |
| Water | 37.25 | 37.25 | 31.95 | 36.25 |
| Hardness (mm) | 5.5 | 6.4 | 4.2 | 5.1 |
| Smear | 9.5 | 9.0 | 8.5 | 8.5 |

### Description of Testing for Examples

### Bar Hardness Test

1. The hardness of a bar is determined by measuring at 25°C the depth of penetration (in mm) into the bar of a 247 gram Standard Weighted Penetrometer Probe having a conically shaped needle attached to a 22.9 cm (9 inch) shaft weighing 47 grams with 200 grams on top of said shaft. A hardness measurement of 5 mm or less indicates a very hard bar; 5-10 mm indicates a moderately hard bar; 10-12 mm indicates a somewhat soft bar of marginal acceptance; and greater than 12 mm indicates a very soft bar that is unacceptable for most uses. This defines "hardness" as used herein unless otherwise specified.

### Bar Smear Test

2. The smear grade is determined by a (1) placing a soap bar on a perch in a 1400 mm diameter circular dish; (2) adding 200 ml of room temperature water to the dish such that the bottom 3 mm of the bar is submerged in water; (3) letting the bar soak overnight (15 hours); (4) turn the bar over and grade qualitatively for the combined amount of smear, and characteristics of smear, depth of smear on a scale where 10 equals no smear, 8.0-9.5 equals low smear amount, 5.0-7.5 equals moderate smears similar to most marketed bars, and 4.5 or less equals very poor smear.
   Commercial soap bars, e.g., SAFEGUARD (RTM), ZEST (RTM), IVORY (RTM), and LAVA (RTM), have smears of about 5, 6, 6, and 6, respectively. See Table 12 for more data.

### Bar Shrinkage Test

3. Shrinkage is measured by placing a freshly made unwrapped bar in a room that is held at 26°C and 15% relative humidity for one week. The amount of shrinkage from the original bar shape is determined on a qualitative scale where 0 indicates no shrinkage, + indicates slight shrinkage, ++ indicates moderate shrinkage, and +++ indicates great shrinkage.
   In Tables 6 and 7, soap bars 1-10 are set out to show bar hardness, smear and shrinkage for C₁₀, C₁₂, C₁₄, C₁₆, and C₁₈ alkyl chain soaps as shown. The preferred alkyl chain soaps of the present invention are set out above in Tables 1 and 2.
   The term "X." means that the example is a comparative example.

**TABLE 6**

| Single Saturated Chain Length Sodium Soap/Water Study | | | | | |
|---|---|---|---|---|---|
| Ingredient | Ex.1 Wt.% | Ex.2 Wt.% | Ex.3 Wt.% | Ex.4 Wt.% | Ex.5 Wt.% |
| Sodium Soap | | | | | |
| C₁₀ | 33 | - | - | - | - |
| C₁₂ | - | 33 | - | - | - |
| C₁₄ | - | - | 33 | - | - |
| C₁₆ | - | - | - | 33 | - |
| C₁₈ | - | - | - | - | 33 |
| Free Fatty Acid | 1.0 | 1.0 | 1.0 | 1.0 | 2.0 |

| Excess Sodium Hydroxide | | | | | |
|---|---|---|---|---|---|
| Sodium Chloride | 2.0 | 1.0 | 1.0 | 1.0 | 1.0 |
| Water | 64 | 65 | 65 | 65 | 64 |
| Hardness (mm) | 8.9 | 2.3 | 2.2 | 5.4 | 4.2 |
| Smear | 3 | 10 | 10 | 9.5 | 10.0 |
| Shrinkage | | +++ | +++ | + | 0 |
| Note that Ex. 1 has a very poor smear, notwithstanding a hardness of 8.9 as the smear methodology dissolves away the soluble C₁₀ soap. | | | | | |

**TABLE 7**

| Single Chain Length Sodium Soap/Water Study | | | | | |
|---|---|---|---|---|---|
| Ingredient | X.6 Wt.% | Ex.7 Wt.% | Ex.8 Wt.% | Ex.9 Wt.% | Ex.10 Wt.% |
| Sodium Soap | | | | | |
| C₁₂ | - | - | - | 15 | 5 |
| C₁₆ | - | 10 | - | - | - |
| C₁₈ | - | - | 10 | - | - |
| C₁₈:1 | 33 | - | - | - | - |
| Free Fatty Acid | 1.0 | - | 2.0 | 1.0 | - |
| Excess Sodium Hydroxide | - | 0.07 | - | - | - |
| Sodium Chloride | 1.0 | 1.0 | 1.0 | 1.0 | 1.0 |
| Water | 65 | 87 | 82.8 | 83 | 94 |
| Hardness (mm) | ** | 11.8 | 11.9 | | 14.0 |
| Smear | | 10.0 | 10.0 | | 9.0 |
| Shrinkage | | 0 | +++ | ++++ | ++++ |

| | | | | | |
|---|---|---|---|---|---|
| ** Solid bar not formed due to too much unsaturated soap. | | | | | |

Example 10 has the rigid structure, but is not preferred as a cleaning bar because its hardness is 14.

**TABLE 8**

| Binary Chain Length Sodium Soap/Water Study | | | |
|---|---|---|---|
| Ingredient | X.11 Wt.% | Ex.12 Wt.% | Ex.13 Wt.% |
| Sodium Soap | | | |
| C₁₀ | - | - | 16.5 |
| C₁₂ | 16.5 | - | - |
| C₁₄ | - | 16.5 | 16.5 |
| C₁₈:1 | 16.5 | 16.5 | - |
| Free Fatty Acid | 1.0 | 1.0 | 1.0 |

| Excess Sodium Hydroxide | | | |
|---|---|---|---|
| Sodium Chloride | 1.0 | 1.0 | 1.0 |
| Water | 65 | 65 | 65 |
| Hardness (mm) | ** | 9.0 | 9.0 |
| Smear | | 9.0 | 8.0 |

| | | | |
|---|---|---|---|
| **Solid Bar not formed due to too much unsaturation combined with C₁₂ soap. | | | |

**TABLE 9**

| Binary Saturated Chain Length Sodium Soap/Water Study | | | |
|---|---|---|---|
| Ingredient | Ex.14 Wt.% | Ex.15 Wt.% | Ex.16 Wt.% |
| Sodium Soap | | | |
| C₁₂ | 16.5 | - | - |
| C₁₄ | 16.5 | - | - |
| C₁₆ | - | 16.5 | 10 |
| C₁₈ | - | 16.5 | 10 |
| Free Fatty Acid | 1.0 | 1.0 | 1.0 |
| Sodium Chloride | 1.0 | 1.0 | 1.0 |
| Water | 65 | 65 | 78 |
| Hardness (mm) | 2.8 | 4.5 | 7.3 |
| Smear | 9.5 | 10.0 | 10.0 |
| Shrinkage | | 0 | ++ |

Examples 12-16 are excellent bars of the present invention.

**TABLE 10**

| Complex Chain Length Sodium Soap/Water Study | | | |
|---|---|---|---|
| Ingredient | Ex.17 Wt.% | Ex.18 Wt.% | Ex.19 Wt.% |
| Sodium Soap* | | | |
| Emersol 132 | - | (33) | (15) |
| C₈ | 0.56 | - | - |
| C₁₀ | 0.64 | - | - |
| C₁₂ | 10.14 | 0.12 | 8.1 (8.0) |
| C₁₄ | 4.54 | 0.79 | 10.4 (10.0) |
| C₁₆ | 8.51 | 15.6 | 7.10 |
| C₁₇ | 0.76 | 0.76 | 0.35 |
| C₁₈ | 19.85 | 15.3 | 7.0 |
| C₂₀ | - | 0.26 | 0.12 |
| Free Fatty Acid | - | 1.0 | - |
| Sodium Chloride | 1.1 | 1.0 | 1.0 |
| Water | 53.9 | 65 | 66 |
| Hardness (mm) | 7.6 | 4.7 | 5.8 |
| Smear | 9.5 | 10 | 9.5 |
| Shrinkage | | + | ++ |

| | | | |
|---|---|---|---|
| *Composition by Chain Length,() indicate actual level of materials. | | | |

Examples 17-19 are made with more complex mixtures of soaps than the prior examples. They form very good bars of the present invention. They have little or no smear. Compare their hardness and smears with those made with conventional tallow and coconut soap shown in Table 11.

**TABLE 11**

| Complex Chain Length Sodium Soap/Water Study | | | |
|---|---|---|---|
| Ingredient | X.20 Wt.% | X.21 Wt.% | X.22 Wt.% |
| Sodium Soap* | | | |
| Tallow | (33) | - | (26.4) |
| Coconut | - | (33) | (6.6) |
| C₈ | - | 2.31 | 0.46 |
| C₁₀ | - | 2.0 | 0.40 |
| C₁₂ | - | 16.5 | 3.3 |
| C₁₄ | 1.0 | 5.94 | 4.95 |
| C₁₆ | 7.92 | 2.81 | 6.90 |
| C₁₈ | 0.5 | - | 0.40 |
| C₂₀ | 6.6 | 1.0 | 5.48 |
| C₁₄:1 | 0.33 | - | 0.26 |
| C₁₆:1 | 0.83 | - | 0.66 |
| C₁₈:1 | 14.2 | 2.0 | 11.76 |
| C₁₈:2 | 0.75 | 0.5 | 0.7 |
| Free Fatty Acid | 1.0 | 1.0 | 1.0 |
| Sodium Chloride | 1.0 | 1.0 | 1.0 |
| Water | 65 | 65 | 65 |
| Hardness (mm) | Soft | 15.8 | 12.5 |
| Smear | Poor | 3.0 | 5.0 |

| | | | |
|---|---|---|---|
| *Composition by Chain Length, () indicate actual level of materials. | | | |

These comparative examples, X.20, X.21, and X.22, do not form the rigid structure of the present invention. Note that they are made with the typical commercial soaps. They are soft soaps with terrible smears. Compare with Example 15 of the present invention which is made with 65% by weight water and C₁₆ and C₁₈ saturated soap and forms a hard bar with no smear.

Example 23 is a bar of the present invention which contains more synthetic surfactant than soap. It has low smear and good lather. Example 24 is a bar of the present invention which contains polymer and other bar soap ingredients.

### EXAMPLE 23

### Syndet Bar Example

| Ingredient | Wt.% |
|---|---|
| Sodium Palmitate | 20 |
| Sodium Lauroyl Sarcosinate | 9* |
| Sodium Laureth-3 Sulfate | 7* |
| Sodium Cetearyl Sulfate | 5* |
| Free Fatty Acid (Palmitic) | 1 |
| Sodium Chloride | 3 |
| Propylene Glycol | 14 |
| Hydrated Zeolite A | 3 |
| Perfume | 1 |
| Water | 37 |

| | |
|---|---|
| *Total 21% Synthetic Surfactant | |

### EXAMPLE 24

### Polymer-Containing Example

| Ingredient | Wt.% |
|---|---|
| Sodium Palmitate | 20 |
| Sodium Alpha-Sulfo Methyl Cocoate | 8.7 |
| Coco Betaine | 4.65 |
| Jaguar C376 | 1.5 |
| Propylene Glycol | 15 |
| Kaolin Clay | 5 |
| Paraffin, (M.P.=55°C) | 4.5 |
| Sodium Chloride | 3 |
| Perfume | 1 |
| Water | 35.5 |

Examples 23 and 24 are similar to Example IV of Table 5.

Example 24 is a mild bar formulation with polymeric skin mildness aid.

### EXAMPLES 25-27

| Ingredient | Ex.25 Wt.% | Ex.26 Wt.% | Ex.27 Wt.% |
|---|---|---|---|
| Lithium Myristate | 33 | - | - |
| Lithium Chloride | 5 | - | - |
| Disodium Salt of Dodecanedioic Acid | - | 20 | 20 |
| Sodium Lauroyl Sarcosinate | - | - | 5 |
| Water | 62 | 80 | 75 |
| Penetration Values | N/A | N/A | N/A |
| N/A = Not available | | | |

For Example 25, the formulation is prepared by heating the fatty acid precursor to 71°C, separately adding lithium hydroxide to water, and then adding the fatty acid and lithium hydroxide solution together, mixing together for 30 minutes maintaining the heat at least at 71°C, adding lithium chloride salt and stirring for an additional 5 minutes, then pouring into a mold and letting cool and solidify. A solid bar with excellent smear properties is formed.

For Examples 26 and 27, the diacid is melted (150-180°C) and a hot (90°C) caustic solution (two equivalents of NaOH) is added. The mixture is stirred for ∼5 minutes. For Example 27, the sodium lauroyl sarcosinate is predissolved in the caustic/water solution. The bar becomes solid on cooling, with further hardening occurring upon degradation, e.g., to 35-40% water by weight of the bar.

Example 25 demonstrates the ability to form high moisture, firm and non-smearing bars without the need for sodium soap. Examples 26 and 27 demonstrate the ability to form a totally soap-free product and still obtain the relatively rigid intermeshed fiber structure.

### FREEZER BAR EXAMPLE 28

Example 28 below is made by a freezer bar process disclosed in commonly assigned, U.S. Pat. Application Ser. No. 07/731,163, Taneri et al., filed July 15, 1991. This process provides a personal cleansing freezer bar comprising a skeleton structure having a relatively rigid, interlocking, semi-continuous, open, three-dimensional, crystalline mesh of neutralized carboxylic acid soap made by the following steps:
(1) mixing a molten mixture comprising by weight of said bar: from 15% to 85% by weight of said soap and from 15% to 40% by weight water;
(2) cooling said mixture to a semi-solid in a scraped wall heat exchanger freezer;
(3) extruding said semi-solid as a soft plug; and
(4) further cooling and crystallizing said soft plug until firm to provide said personal cleansing freezer bar.

### Step 1 - Mixing

The soap specified in the formulation is made in situ by mixing the desired fatty acids, consisting essentially of C₁₂-C₂₄ chain lengths, with the appropriate base or mixture of bases, consisting essentially of sodium, lithium, magnesium, calcium, and potassium hydroxide and triethanolamine. The fatty acid, base, and water are mixed at from about 170°F to about 200°F (76°-93°C) to form the soap. In Example 28, 180°F is used. Sufficient water is used such that the mixture is stirrable. The other ingredients are added, maintaining the temperature of from about 180°F to about 200°F (82°-93°C). Example 28 - 180°F. The optimal mixing temperatures can vary depending on the particular formulation.

### Step 2 Optionals - Aeration, Minor Addition, and Flash Drying Optionals

Aerate (optional) said mix and add perfume (only if drying) and other minors with positive displacement pump or other in-line mixer. Example 28 is not aerated or dried. The mixture of Step (1) is optionally dried to reduce the amount of said water to the desired level, preferably 20-40% by weight water. The flash drying temperature is from about 225°F to about 315°F (135°-157°C) at pressure of from about 30 to abut 100 psi (115-517 mm Hg).

### Step 3 - Freezer

Cool the mix using a scraped wall heat exchanger (freezer) to partially crystallize the components from an initial temperature of from about 180°F to about 200°F (82°-93°C) or from about 200°F to about 220°F (93°-104°C), if dried, to a final temperature preferably from about 135°F to about 180°F (57°-82°C), more preferably from about 145°F to about 180°F (63°-82°C), and most preferably from about 155°F to about 175°F (68°-79°C). This final temperature, also referred to herein as the Freezer Outlet Temperature (FOT), is typically the maximum temperature that will form a smooth plug that holds its shape once extruded onto a moving belt (Step 4). The FOT for Example 28 is 175°F.

### Step 4 - Extrusion

The cooled mix of Step 3 is extruded out onto a moving belt as a soft plug which is then cooled and fully crystallized and then stamped and packaged. The plugs are preferably formed via an extrusion operation, as shown in US-A-3,835,059, supra. Some of the composition crystallizes in the freezer (Step 3) in order to provide a semi-solid having a sufficient viscosity to stand up on the belt, while further crystallization occurs after extrusion, resulting in hardening of the bar. The final crystallization of the sodium soap forms the interlocking, semi-continuous, open mesh structure in the freezer bar of the present invention.

### EXAMPLE 28

| Ingredient | Wt.% |
|---|---|
| Sodium C₁₄ Soap | 27.99 |
| Magnesium C₁₄ Soap | 5.00 |
| Sodium Lauroyl Sarcosinate | 3.00 |
| Coco Betaine | 10.00 |
| Propylene Glycol | 3.50 |
| Petrolatum | 22.49 |
| Sodium Chloride | 2.58 |
| Free Fatty Acid, C₁₄ | 0.50 |
| Perfume | 0.50 |
| Water | 24.44 |

### The Plodding Stamped Bar Hardness Test

The Plodding Stamped Bar Hardness Test can be used to differentiate the bars of this invention from other bars. Four trade bars are selected that represent various soap processes: SAFEGUARD (RTM), a soap milled bar; ZEST (RTM), a soap synthetic milled bar; IVORY (RTM), a freezer bar; and LAVA (RTM), a framed bar. Samples of these market bars and formed bars of Example 28 and Example II are plodded using the procedure set out below.

Overall, the market bars after plodding are much harder and have a better smear versus Example 28 or Example II after plodding. This data is detailed in Table 12. This test clearly is an excellent method of differentiating bars containing the rigid skeletal structure versus other bars. Simply stated, the bars of this invention will become much more soft after replodding than conventional bars.

The procedure is as follows:
1. Formed bars (about 2.5 Kg or greater) are placed into a single stage plodder (4 inch/10.16 cm bonnet single stage plodder) without vacuum and are run through a noodle plate. The noodle plate contains nineteen 0.37 inch (0.93 cm) holes in a 3.1 inch (8 cm) plate. The barrel temperature is set at 120°F (49°C) and the nose temperature is set at 110°F (43.5°C).
2. Step 1 is repeated with the noodles.
3. The noodles of Step 2 are placed into the single stage plodder (4 inch/10.16 cm bonnet single stage plodder) with vacuum applied and run through a brick-shaped orifice. A brick-shaped plug with approximate dimensions of 1.88 inches (4.6 cm) (height) by 1.16 inches (3 cm) (width) by 3 inches (7.6 cm) (length) is extruded. These plugs should have an interior temperature of 90°F (32°C) to 105°F (41°C).
4. These plugs are stamped into a brick shape and are allowed to cool to room temperature (at least 12 hours) before evaluation.

**TABLE 12**

| Bar Plodder Data | |
|---|---|
| Bar | Hardness (mm)* |
| 1 SAFEGUARD (RTM) Market Bar | 3.18 |
| 2 SAFEGUARD (RTM) (Plodded/Stamped) | 3.13 |
| Delta (The value of Bar 1-Bar 2) | 0.05 |
| 1 ZEST (RTM) Market Bar | 2.25 |
| 2 ZEST (RTM) (Plodded/Stamped) | 2.33 |
| Delta | (0.08) |
| 1 IVORY (RTM) Market Bar | 1.93 |
| 2 IVORY (RTM) (Plodded/Stamped) | 3.03 |
| Delta | (1.10) |
| 1 LAVA (RTM) Market Bar | 1.90 |
| 2 LAVA (RTM) (Plodded/Stamped) | 2.47 |
| Delta | (0.57) |
| 1 Example 28 (Formed Bar) | 3.35 |
| 2 Example 28 (Plodded/Stamped) | 10.67 |
| Delta | (7.32) |
| 1 Example II (Formed Bar) | 6.43 |
| 2 Example II (Plodded/Unstamped) | 18.07 |
| Delta | (11.64) |

| | |
|---|---|
| *The "hardness" of the "plodder/stamped" bars is reported as Bar 2 in Table 12 for each bar tested. The Bar Hardness lest is set out herein elsewhere. | |

While not being bound to a theory, plodded bars with Delta's of 4 or greater is a strong indication that there is a skeletal structure in the original which is fractured or destroyed when plodded. The hard bars of the present invention will form soft, messy bars when plodded in a conventional bar process.

The bars of Example 28 bars are first formed using the above freezer process. The bars of Example II are first formed using the above-described frame bar process.

About 5-10 Kg of each bar is plodded and stamped.

The market bars are made of tallow and coconut natural soaps. The hardness of plodded SAFEGUARD (RTM) and ZEST (RTM) bars are about the same as the original bars. The IVORY (RTM) and LAVA (RTM) plodded bars (2) are slightly softer than the original bars.

On the other hand, the plodded Bar 2 of Example 28 is much softer than the original Bar 1 of Example 28. More dramatically, the plodded Bar 2 of Example II falls apart upon plodding and is too soft to stamp. Its hardness after plodding is that of a soft aqueous phase, indicating that the rigidity of the skeletal structure is essentially destroyed.

## Claims

1. A non-transparent cleansing bar comprising at least two phases:
an aqueous phase having a penetration value of 12 mm for a 12 mm deep sample; said aqueous phase being soft or flowable at 25°C;
a rigid crystalline phase skeleton structure comprising an interlocking, open three-dimensional mesh of neutralized mono-and/or di-carboxylic acid elongated light diffracting crystals having a diameter or length greater than 400nm;
wherein said cleansing bar comprising said rigid crystalline phase skeleton structure and said aqueous phase has a penetration value of of from zero to about 12 mm for a 25 mm deep sample of said cleansing bar;
wherein said penetration values are measured as 25°C using a 247 gram Standard Weighted Penetrometer Probe having a conical needle attached to a 9 inch (22.9 cm) shaft, weighing 47 grams with 200 grams on top of said shaft for a total of said 247 grams, said conical needle having a 19/32 inch (1.51 cm) top and a 1/32 inch (0.08 cm) point;
wherein said neutralized carboxylic acid is selected from the group consisting of: lithium and/or sodium neutralized: monocarboxylic acid (soap) and/or dicarboxylic acid; and mixtures thereof;
wherein said monocarboxylic acid has a fatty alkyl(ene) chain of from about 12 to about 24 carbon atoms;
wherein said dicarboxylic acid has a fatty alkyl(ene) chain of from about 12 to about 18 carbon atoms; and
wherein at least 80% of said carboxylic acid has saturated alkyl chains;
wherein said rigid crystalline phase skeleton structure occupies from 3% to 75% of said cleansing bar by volume;
and
wherein said neutralized carboxylic acid comprises from over 5% to 75% by weight of said cleansing bar; and
wherein said cleansing bar contains from 15% to 94% by weight water.

2. The cleansing bar of Claim 1 wherein at least 80% of said carboxylic acid has the following general formula: wherein:$\text{a + b = 8 to 20}$ each a, b = 0 to 20
X = H, OR, R, or mixtures thereof
R = C₁-C₃ alkyl, H, or mixtures thereof
M = Na, Li, or mixtures thereof.

3. The cleansing bar of Claim 2 wherein said $\text{a + b = 10-16}$ ; each of said a, b = 0-16; said X = H, OR; R = H; and M = Na.

4. The cleansing bar of Claim 3 wherein said elongated crystals are composed of fiber-like sodium fatty acid soap of which at least 25% of said saturated fatty alkyl chains is of a single chain length; and wherein said bar contains: from 15% to 75% by weight of said sodium soap; wherein said bar contains unneutralized (free) carboxylic acid of no more than 50% by weight of said soap; and preferably wherein said bar contains said sodium soap and water; and from 2% to 60% by weight of a synthetic surfactant selected from the group consisting of: alkyl sulfates, paraffin sulfonates, alkylglycerylether sulfonates, acyl sarcosinates, methylacyl taurates, linear alkyl benzene sulfonates, N-acyl glutamates, alkyl glucosides, alpha sulfo fatty acid esters, acyl isethionates, alkyl sulfosuccinates, alkyl ether carboxylates, alkyl phosphate esters, ethoxylated alkyl phosphate esters, methyl glucose esters, protein condensates, alkyl amine oxides, alkyl betaines, alkyl sultaines, the alkyl ether sulfates with 1 to 12 ethoxy groups, and mixtures thereof, wherein said surfactants contain C₈-C₂₂ alkyl chains.

5. The cleansing bar of Claim 4 wherein said synthetic surfactant is hygroscopic; said hygroscopic surfactant being defined as a surfactant which absorbs at least 20% of its dry weight in water at 26°C and 80% Relative Humidity in three days and wherein said bar is relatively non-swelling; and preferably wherein said hygroscopic surfactant is selected from the group consisting of alpha sulfo fatty acid esters; alkyl sulfates; alkyl ether carboxylates; alkyl betaines; alkyl sultaines; alkyl amine oxides; alkyl ether sulfates; and mixtures thereof.

6. The cleansing bar of Claim 4 or 5 wherein the ratio of said water to said soap is from about 1:1 to about 5:1; said water is present at a level of from 25% to 60% by weight; wherein said soap has fatty alkyl chains are C₁₄ to C₂₂ and said soap level in said bar is from 15% to 35% by weight; wherein at least 85% of said soap alkyl chains are saturated; wherein said unneutralized (free) carboxylic acid is from zero to about 25% by weight of said soap; and wherein said synthetic surfactant level is from 4% to 25% by weight of the bar and said surfactant is selected from the group consisting of: sodium acyl isethionates, sodium acyl sarcosinates, sodium alpha sulfo fatty acid esters, sodium paraffin sulfonates, sodium alkyl ether sulfates, sodium alkyl sulfates, sodium linear alkyl benzene sulfonates, alkyl betaines, alkyl sultaines, and trialkyl amine oxides; and preferably wherein the ratio of said water to soap ratio is from about 1.5:1 to about 2:1; said unneutralized (free) carboxylic acid is from zero to 17% by weight of said soap; said water level is from 30% to 45% by weight; said soap fatty alkyl chain is from about C₁₄ to about C₁₈; wherein at least 95% of said alkyl chains are saturated; said soap level is from 15% to 30% by weight; and said synthetic surfactant level is from 8% to 16% by weight.

7. The cleansing bar of Claim 5 or 6 wherein said bar contains from 0.1% to 40% by weight of a hydrophobic material selected from the group consisting of: microcrystalline wax, petrolatum, carnauba wax, palm wax, candelilla wax, sugarcane wax, vegetable derived triglycerides, beeswax, spemaceti, lanolin, wood wax, shellac wax, animal derived triglycerides, montar, ozokerite, ceresin, and Fischer-Tropsch wax; and preferably wherein said bar contains from 2% to 35% by weight of said hydrophobic material selected from the group consisting of petrolatum and wax, said petrolatum and wax, and mixtures thereof having a melting point of from about 49°C (120°F) to about 85°C (185°F); and more preferably wherein said bar comprises from 5% to 25% by weight of the bar of paraffin wax; and wherein said bar contains from 1% to 50% by weight of a non-volatile, water-soluble, nonionic organic material having a solubility of at least 5 parts in 10 parts of water; and wherein said water-soluble nonionic organic material is selected from the group consisting of a polyol of the structure: where R₁ = H, C₁-C₄ alkyl; R₂ = H, CH₃; and n = 1-200;
C₂-C₁₀ alkane diols; sorbitol; glycerine; sugars; sugar derivatives; urea; and
ethanol amines of the general structure (HOCH₂CH₂)ₓNH_{y} where x = 1-3; y = 0-2; and x+y = 3, and mixtures thereof; and preferably wherein said non-volatile, water-soluble, nonionic organic material comprises from 5% to 20% by weight of the bar; when said organic material is selected from the group consisting of: propylene glycol, glycerine, sucrose, and urea, and mixtures thereof.

8. The cleansing bar of Claim 5, 6 or 7 wherein said bar contains said sodium soap, said water, and said synthetic surfactant, and from 0.1% to 70% by weight of other ingredients selected from the group consisting of:
from 1% to 10% said potassium soap;
from 1% to 35% said magnesium soap;
from 1% to 35% by weight said calcium soap;
from 1% to 15% by weight triethanolammonium soap;
from 1% to 60% by weight of impalpable water-insoluble materials selected from the group consisting of calcium carbonate and talc;
from 0.1% to 20% by weight of a polymeric skin feel aid;
from 0.5% to 25% by weight of aluminosilicate clay and/or other clays; wherein said aluminosilicates and clays are selected from the group consisting of zeolites; kaolin, kaolinite, montmorillonite, attapulgite, illite, bentonite, halloysite, and calcined clays;
from 1% to 50% by weight of salt and salt hydrates; and mixtures thereof; and wherein said salt and salt hydrate have a cation selected from the group consisting of: sodium, potassium, magnesium, calcium, aluminum, lithium, ammonium, monoethanol ammonium, diethanolammonium, and triethanolammonium; and wherein said salt and salt hydrate have an anion selected from the group consisting of: chloride, bromide, sulfate, metasilicate, orthophosphate, pyrophosphate, polyphosphate, metaborate, tetraborate, carbonate, bicarbonate, hydrogen phosphate, methyl sulfate, and mono- and polycarboxylate of 6 carbon atoms or less.

9. The process of making a cleansing bar of Claim 1-8 said process comprising the steps of:
I. forming an aqueous molten liquid comprising from 20% to 94% by weight water and from about greater than 5% to 75% by bar weight said neutralized carboxylic acid;
II. pouring said molten liquid into a bar shaped mold; and
III. crystallizing said molded molten liquid by cooling to provide said cleansing bar; preferably
wherein the aqueous molten liquid is made by neutralizing an aqueous mixture of said carboxylic acid with a hydroxide selected from the group consisting of sodium hydroxide or lithium hydroxide and mixtures thereof with stirring at a temperature of from about 50°C (120°F) to about 95°C (205°F); and said molten liquid contains from 2% to 15% by weight of said bar of a "crystallization enhancing salt" selected from the group consisting of: sodium or lithium salt of sulfate, chloride, acetate and citrate, and mixtures thereof; and preferably when said aqueous molten liquid aqueous phase contains from 2% to 40% of a solubilizing aid, said solubilizing aid is selected from the group consisting of:
(a) non-volatile, water-soluble nonionic organic solvents selected from the group consisting of: a polyol of the structure: where R₁ = H, C₁-C₄ alkyl; R₂ = H, CH₃; and n = 1-200; C₂-C₁₀ alkane diols; sorbitol; glycerine; sugars; sugar derivatives; urea; and ethanol amines of the general structure (HOCH₂CH₂)ₓNH_{y} where x = 1-3; y = 0-2; and x+y = 3;
(b) alcohols of from 1 to 5 carbon atoms;
(c) synthetic surfactant selected from the group consisting of: alkyl sulfates, paraffin sulfonates, alkyl glyceryl ether sulfonates, anionic acyl sarcosinates, methyl acyl taurates, linear alkyl benzene sulfonates, N-acyl glutamates, alkyl glucosides, alpha sulfo fatty acid esters, acyl isethionates, alkyl sulfosuccinates, alkyl ether carboxylates, alkyl phosphate esters, ethoxylated alkyl phosphate esters, methyl glucose esters, protein condensates, alkyl amine oxides, alkyl betaines, alkyl sultaines, the alkyl ether sulfates with 1 to 12 ethoxy groups, and mixtures thereof, wherein said surfactants contain C₈-C₂₂ alkylene chains; and mixtures thereof; and
wherein said solubilizing aid is added to increase the level of said neutralized carboxylic acid dissolved in said continuous molten aqueous phase in step I.

10. The process of Claim 9 wherein said aqueous phase contains from 20% to 100% water by weight of said aqueous phase; and wherein said rigid crystalline phase contains from 75% to 100% of said neutralized carboxylic acid by weight of said crystalline phase; and wherein said bar has a penetration value of from 3 mm to 9 mm for said 25 mm bar sample.

11. A personal cleansing bar composition according to claim 1 comprising a rigid, crystalline interlocking open three dimensional mesh of elongated sodium soap crystals having a diameter or length greater than 400nm; said soap bar comprising: from 15% to 50% by weight sodium fatty acid soap composed of at least 50% saturated fatty alkylene chains having 12-24 carbon atoms of which at least 25% of said saturated fatty alkyl chains is of a single chain length; from 15% to 60% by weight water; and from 2% to 60% by weight of a hygroscopic synthetic surfactant wherein said hygroscopic synthetic surfactant is selected from surfactants which absorb at least 20% of their dry weight in water at 26°C and 80% Relative Humidity in three days.

12. The personal cleansing bar of Claim 11 wherein said hygroscopic synthetic surfactant is selected from the group consisting of alpha sulfo fatty acid esters; alkyl sulfates; alkyl ether carboxylates; alkyl betaines; alkyl sultaines; alkyl amine oxides; alkyl ether sulfates; and mixtures thereof; and wherein said bar contains from 0.5% to 40% by weight of salts and/or salt hydrates selected from the group consisting of: sodium chloride, sodium sulfate, disodium hydrogen phosphate, sodium pyrophosphate, sodium tetraborate, sodium acetate, sodium citrate, and other compatible salts of inorganic acids and short chain organic acids.

## Patentansprüche

1. Nicht-transparenter Reinigungsriegel, welcher mindestens zwei Phasen umfaßt:
eine wäßrige Phase mit einem Penetrationswert von 12 mm bei einer 12 mm starken Probe; welche wäßrige Phase bei 25°C weich oder fließfähig ist;
eine rigide, eine kristalline Phase bildende Skelettstruktur, umfassend ein ineinandergreifendes, offenes, dreidimensionales Netz aus langgestreckten, das Licht beugenden Kristallen aus neutralisierter Mono- und/oder Dicarbonsäure mit einem Durchmesser oder einer Länge von mehr als 400 nm;
wobei der genannte Reinigungsriegel, welcher die genannte rigide, eine kristalline Phase darstellende Skelettstruktur und die genannte wäßrige Phase umfaßt, einen Penetrationswert von Null bis etwa 12 mm bei einer 25 mm starken Probe des genannten Reinigungsriegels aufweist;
wobei die genannten Penetrationswerte bei 25°C unter Verwendung einer Penetrometersonde mit einem Eichgewicht (Standard Weighted Penetrometer Probe) von 247 Gramm ermittelt werden, welche Sonde eine an einem Schaft von 9 Inch (22,9 cm) befestigte Nadel aufweist, die 47 Gramm wiegt, mit 200 Gramm am oberen Ende des genannten Schaftes, um insgesamt die genannten 247 Gramm zu erreichen, welche konische Nadel eine Basis von 19/32 Inch (1,51 cm) und eine Spitze von 1/32 Inch (0,08 cm) besitzt;
wobei die genannte neutralisierte Carbonsäure von der Gruppe ausgewählt ist, welche aus mit Lithium und/oder mit Natrium neutralisierter Monocarbonsäure (Seife) und/oder Dicarbonsäure und Gemischen hievon besteht;
wobei die genannte Monocarbonsäure eine Fettalkyl(en)kette von etwa 12 bis etwa 24 Kohlenstoffatomen aufweist;
wobei die genannte Dicarbonsäure eine Fettalkyl(en)kette von etwa 12 bis etwa 18 Kohlenstoffatomen besitzt; und
wobei mindestens 80% der genannten Carbonsäure gesättigte Alkylketten aufweisen;
wobei die genannte rigide, eine kristalline Phase bildende Skelettstruktur 3% bis 75% des genannten Reinigungsriegels, bezogen auf das Volumen, umfaßt; und
wobei die genannte neutralisierte Carbonsäure über 5 Gew.-% bis 75 Gew.-% des genannten Reinigunsriegels darstellt; und
wobei der genannte Reinigungsriegel 15 Gew.-% bis 94 Gew.-% Wasser enthält.

2. Reinigungsriegel nach Anspruch 1, worin mindestens 80% der genannten Carbonsäure die folgende allgemeine Formel: besitzen, worin:$\text{a + b von 8 bis 20 beträgt,}$ jedes a, b von 0 bis 20 ist,
X für H, OR, R oder Gemische hievon steht,
R C₁-C₃-Alkyl, H oder Gemische hievon bedeutet,
M Na, Li oder Gemische hievon darstellt.

3. Reinigungsriegel nach Anspruch 2, worin a + b von 10 bis 16 ist; jedes a, b von 0 bin 16 beträgt; das genannte X für H, OR steht; R H bedeutet; und M Natrium darstellt.

4. Reinigungsriegel nach Anspruch 3, worin die genannten langgestreckten Kristalle aus faserartiger Natriumfettsäureseife zusammengesetzt sind, wobei mindestens 25% der genannten gesättigten Fettalkylketten eine einzige Kettenlänge aufweisen; und wobei der genannte Riegel 15 Gew.-% bis 75 Gew.-% der genannten Natriumseife enthält; wobei der genannte Riegel nicht neutralisierte (freie) Carbonsäure in einer Menge von nicht mehr als 50%, bezogen auf das Gewicht der genannten Seife, umfaßt; und vorzugsweise der genannte Riegel Natriumseife und Wasser enthält; und 2 Gew.-% bis 60 Gew.-% eines synthetischen grenzflächenaktiven Mittels umfaßt, welches von der aus Alkylsulfaten, Paraffinsulfonaten, Alkylglycerylethersulfonaten, Acylsarcosinaten, Methylacyltauraten, linearen Alkylbenzolsulfonaten, N-Acylglutamaten, Alkylglucosiden, alpha-Sulfofettsäureestern, Acylisethionaten, Alkylsulfosuccinaten, Alkylethercarboxylaten, Alkylphosphatestern, ethoxylierten Alkylphosphatestern, Methylglucoseestern, Proteinkondensaten, Alkylaminoxiden, Alkylbetainen, Alkylsultainen, den Alkylethersulfaten mit 1 bis 12 Ethoxygruppen, und Gemischen hievon bestehenden Gruppe ausgewählt ist, wobei die genannten grenzflächenaktiven Mittel C₈-C₂₂-Alkylketten aufweisen.

5. Reinigungsriegel nach Anspruch 4, worin das genannte synthetische grenzflächenaktive Mittel hygroskopisch ist; welches hygroskopische grenzflächenaktive Mittel als ein grenzflachenaktives Mittel definiert ist, das bei 26°C und 80% relativer Feuchtigkeit in drei Tagen mindestens 20% seines Trockengewichtes an Wasser absorbiert, und wobei der genannte Riegel verhältnismäßig nicht-quellend ist; und wobei das genannte hygroskopische grenzflächenaktive Mittel vorzugsweise von der aus alpha-Sulfofettsäureestern; Alkylsulfaten; Alkylethercarboxylaten; Alkylbetainen; Alkylsultainen; Alkylaminoxiden; Alkylethersulfaten; und Gemischen hievon bestehenden Gruppe ausgewählt ist.

6. Reinigungsriegel nach Anspruch 4 oder 5, worin das Verhältnis vom genannten Wasser zur genannten Seife von etwa 1:1 bis etwa 5:1 beträgt; welches Wasser in einer Menge von 25 Gew.-% bis 60 Gew.-% vorhanden ist; wobei die genannte Seife Fettalkylketten von C₁₄ bis C₂₂ aufweist und die genannte Seifenmenge im genannten Riegel von 15 Gew.-% bis 35 Gew.-% beträgt; wobei mindestens 85% der genannten Seifenalkylketten gesättigt sind; wobei die genannte nicht-neutralisierte (freie) Carbonsäure Null bis etwa 25 Gew.-% der genannten Seife bildet; und wobei die Menge des genannten synthetischen grenzflächenaktiven Mittels 4 Gew.-% bis 25 Gew.-% des Riegels beträgt und das genannte grenzflächenaktive Mittel von der aus Natriumacylisethionaten, Natriumacylsarcosinaten, Natrium-alpha-sulfofettsäureestern, Natriumparaffinsulfonaten, Natriumalkylethersulfaten, Natriumalkylsulfaten, linearen Natriumalkylbenzolsulfonaten, Alkylbetainen, Alkylsultainen und Trialkylaminoxiden bestehenden Gruppe ausgewählt ist; und vorzugsweise das Verhältnis des genannten Verhältnisses von Wasser zu Seife von etwa 1,5:1 bis etwa 2:1 beträgt; die genannte nicht-neutralisierte (freie) Carbonsäure Null bis 17 Gew.-% der genannten Seife darstellt; die genannte Wassermenge 30 Gew.-% bis 45 Gew.-% beträgt: die genannte Seifenfettalkylkette von etwa C₁₄ bis etwa C₁₈ ist; wobei mindestens 95% der genannten Alkylketten gesättigt sind; wobei die genannte Seifenmenge 15 Gew.-% bis 30 Gew.-% beträgt; und die Menge des genannten synthetischen grenzflächenaktiven Mittels 8 Gew.-% bis 16 Gew.-% ist.

7. Reinigungsriegel nach Anspruch 5 oder 6, wobei der genannte Riegel 0,1 Gew.-% bis 40 Gew.-% eines hydrophoben Materials umfaßt, welches von der aus mikrokristallinem Wachs, Petrolatum, Carnaubawachs, Palmwachs, Candelillawachs, Zuckerrohrwachs, aus Pflanzen stammenden Triglyceriden, Bienenwachs, Spemaceti, Lanolin, Holzwachs, Schellackwachs, aus Tieren stammenden Triglyceriden, Montar, Ozokerit, Ceresin und Fischer-Tropsch-Wachs bestehenden Gruppe ausgewählt ist; und vorzugsweise der genannte Riegel 2 Gew.-% bis 35 Gew.-% des genannten hydrophoben Materials umfaßt, welches von der aus Petrolatum und Wachs bestehenden Gruppe ausgewählt ist, wobei Petrolatum und Wachs und die Gemische hievon einen Schmelzpunkt von etwa 49°C (120°F) bis etwa 85°C (185°F) aufweisen; und stärker bevorzugt der genannte Riegel 5% bis 25%, bezogen auf das Gewicht des Riegels, an Paraffinwachs enthält; und wobei der genannte Riegel 1 Gew.-% bis 50 Gew.-% eines nichtflüchtigen, wasserlöslichen, nichtionischen organischen Materials mit einer Löslichkeit von mindestens 5 Teilen in 10 Teilen Wasser aufweist; und wobei das genannte wasserlösliche, nichtionische organische Material von der Gruppe ausgewählt ist, welche aus einem Polyol der Struktur: worin R₁ H oder C₁-C₄-Alkyl bedeutet, R₂ für H, CH₃ steht, und n einen Wert von 1 bis 200 aufweist; C₂-C₁₀-Alkandiolen; Sorbit; Glycerin; Zuckern; Zuckerderivaten; Harnstoff; und Ethanolaminen der allgemeinen Struktur (HOCH₂CH₂)ₓNH_{y}, worin x von 1 bis 3 ist; y von 0 bis 2 beträgt; und x+y gleich 3 ist, und Gemischen hievon besteht; und wobei das genannte nichtflüchtige, wasserlösliche, nichtionische organische Material vorzugsweise 5 Gew.-% bis 20 Gew.-% des Riegels darstellt, wenn das genannte organische Material von der aus Propylenglykol, Glycerin, Saccharose, Harnstoff und Gemischen hievon bestehenden Gruppe ausgewählt ist.

8. Reinigungsriegel nach Anspruch 5, 6 oder 7, worin der genannte Riegel die genannte Natriumseife, das genannte Wasser und das genannte synthetische grenzflächenaktive Mittel und 0,1 Gew.-% bis 70 Gew.-% an anderen Bestandteilen enthält, welche von der Gruppe ausgewählt sind, die aus:
1% bis 10% der genannten Kaliumseife;
1% bis 35% der genannten Magnesiumseife;
1 Gew.-% bis 35 Gew.-% der genannten Calciumseife;
1 Gew.-% bis 15 Gew.-% Triethanolammoniumseife;
1 Gew.-% bis 60 Gew.-% von äußerst feinen, wasserunlöslichen Materialien, welche von der aus Calciumcarbonat und Talk bestehenden Gruppe ausgewählt sind;
0,1 Gew.-% bis 20 Gew.-% von einem polymeren Hilfsmittel für das Anfühlen der Haut;
0,5 Gew.-% bis 25 Gew.-% von Aluminosilicatton und/oder anderen Tonen; wobei die genannten Aluminosilicate und Tone von der aus Zeolithen; Kaolin, Kaolinit, Montmorillonit, Attapulgit, Illit, Bentonit, Halloysit und calcinierten Tonen bestehenden Gruppe ausgewählt sind;
1 Gew.-% bis 50 Gew.-% von Salz und Salzhydraten; und Gemischen hievon besteht; und wobei das genannte Salz und das genannte Salzhydrat ein Kation aufweisen, welches von der aus Natrium, Kalium, Magnesium, Calcium, Aluminium, Lithium, Ammonium, Monoethanolammonium, Diethanolammonium und Triethanolammonium bestehenden Gruppe ausgewählt ist; und worin das genannte Salz und das genannte Salzhydrat ein Anion aufweisen, welches von der aus Chlorid, Bromid, Sulfat, Metasilicat, Orthophosphat, Pyrophosphat, Polyphosphat, Metaborat, Tetraborat, Carbonat, Bicarbonat, Hydrogenphosphat, Methylsulfat und Mono- und Polycarboxylat mit 6 Kohlenstoffatomen oder weniger, bestehenden Gruppe ausgewählt ist.

9. Verfahren zur Herstellung eines Reinigungsriegels nach Anspruch 1 bis 8, welches Verfahren die Schritte von:
I. Ausbilden einer wäßrigen geschmolzenen Flüssigkeit, welche 20 Gew.-% bis 94 Gew.-% Wasser und von mehr als etwa 5% bis 75%, bezogen auf das Gewicht des Riegels, von der genannten neutralisierten Carbonsäure umfaßt;
II. Leeren der genannten geschmolzenen Flüssigkeit in eine Riegel-Form; und
III. Kristallisieren der genannten geformten geschmolzenen Flüssigkeit durch Abkühlen, um den genannten Reinigungsriegel zu erhalten; vorzugsweise
wobei die wäßrige geschmolzene Flüssigkeit durch Neutralisieren eines wäßrigen Gemisches aus der genannten Carbonsäure mit einem Hydroxid, welches von der aus Natriumhydroxid oder Lithiumhydroxid und Gemischen hievon bestehenden Gruppe ausgewählt ist, unter Rühren bei einer Temperatur von etwa 50°C (120°F) bis etwa 95°C (205°F) hergestellt wird; und wobei die genannte geschmolzene Flüssigkeit 2% bis 15%, bezogen auf das Gewicht des genannten Riegels, von einem die "Kristallisation erhöhenden Salz" enthält, welches von der aus Natrium- oder Lithiumsulfat-, -chlorid-, -acetat- und -citratsalzen, und Gemischen hievon bestehenden Gruppe ausgewählt ist; und vorzugsweise die, die genannte wäßrige Phase bildende wäßrige geschmolzene Flüssigkeit 2% bis 40% eines Solubilisierungshilfsmittels umfaßt, welches Solubilisierungshilfsmittel von der Gruppe ausgewählt ist, die aus:
(a) nicht-flüchtigen, wasserlöslichen, nichtionischen organischen Lösungsmitteln, welche von der Gruppe ausgewählt sind, die aus einem Polyol der Struktur: worin R₁ für H oder C₁-C₄-Alkyl steht, R₂ H, CH₃ bedeutet, und n einen Wert von 1 bis 200 besitzt; C₂-C₁₀-Alkandiolen; Sorbit; Glycerin; Zuckern, Zuckerderivaten; Harnstoff; und Ethanolaminen der allgemeinen Struktur (HOCH₂CH₂)ₓNH_{y} besteht, worin x von 1 bin 3 ist; y von 0 bis 2 beträgt; und x+y 3 ist;
(b) Alkoholen mit 1 bis 5 Kohlenstoffatomen;
(c) synthetischem grenzflächenaktivem Mittel, welches von der aus Alkylsulfaten, Paraffinsulfonaten, Alkylglycerylethersulfonaten, anionischen Acylsarcosinaten, Methylacyltauraten, linearen Alkylbenzolsulfonaten, N-Acylglutamaten, Alkylglucosiden, alpha-Sulfofettsäureestern, Acylisethionaten, Alkylsulfosuccinaten, Alkylethercarboxylaten, Alkylphosphatestern, ethoxylierten Alkylphosphatestern, Methylglucoseestern, Proteinkondensaten, Alkylaminoxiden, Alkylbetainen, Alkylsultainen, den Alkylethersulfaten mit 1 bis 12 Ethoxygruppen, und Gemischen hievon, bestehenden Gruppe ausgewählt ist, wobei die genannten grenzflächenaktiven Mittel C₈-c₂₂-Alkylenketten besitzen;
und Gemischen hievon besteht;
und wobei das genannte Solubilisierungshilfsmittel zugesetzt wird, um die Menge der genannten neutralisierten Carbonsäure, die in der genannten kontinuierlichen, geschmolzenen, wäßrigen Phase im Schritt I gelöst ist, zu erhöhen.

10. Verfahren nach Anspruch 9, wobei die genannte wäßrige Phase 20% bis 100% Wasser, bezogen auf das Gewicht der genannten wäßrigen Phase, enthält; und wobei die genannte rigide kristalline Phase 75% bis 100% der genannten neutralisierten Carbonsäure, bezogen auf das Gewicht der genannten kristallinen Phase, umfaßt; und wobei der genannte Riegel einen Penetrationswert von 3 mm bis 9 mm bei der genannten Riegelprobe von 25 mm aufweist.

11. Riegelzusammensetzung für die Körperreinigung nach Anspruch 1, welche ein rigides kristallines, ineinandergreifendes, offenes, dreidimensionales Netz aus langgestreckten Kristallen mit einem Durchmesser oder einer Länge von mehr als 400 nm aus Natriumseife umfaßt; welcher Seifenriegel 15 Gew.-% bis 50 Gew.-% Natriumfettsäureseife mit mindestens 50% gesättigten Fettalkylenketten mit 12 bis 24 Kohlenstoffatomen, wovon mindestens 25% der genannten gesättigten Fettalkylketten eine einzige Kettenlänge aufweisen; 15 Gew.-% bis 60 Gew.-% Wasser; und 2 Gew.-% bis 60 Gew.-% von einem hygroskopischen, synthatischen grenzflächenaktiven Mittel umfaßt, wobei das genannte hygroskopische, synthetische grenzflächenaktive Mittel unter grenzflächenaktiven Mitteln ausgewählt ist, welche bei 26°C und 80% relativer Feuchtigkeit in drei Tagen mindestens 20% ihres Trockengewichtes an Wasser absorbieren.

12. Riegel für die Körperreinigung nach Anspruch 11, wobei das genannte hygroskopische, synthetische grenzflächenaktive Mittel von der aus alpha-Sulfofettsäureestern; Alkylsulfaten; Alkylethercarboxylaten; Alkylbetainen; Alkylsultainen; Alkylaminoxiden; Alkylethersulfaten; und Gemischen hievon bestehenden Gruppe ausgewählt ist; und wobei der genannte Riegel 0,5 Gew.-% bis 40 Gew.-% an Salzen und/oder Salzhydraten umfaßt, welche von der aus Natriumchlorid, Natriumsulfat, Dinatriumhydrogenphosphat, Natriumpyrophosphat, Natriumtetraborat, Natriumacetat, Natriumcitrat und anderen verträglichen Salzen von anorganischen Säuren und kurzkettigen organischen Säuren bestehenden Gruppe ausgewählt sind.

## Revendications

1. Pain nettoyant non transparent, comprenant au moins deux phases:
une phase aqueuse ayant un indice de pénétration de 12 mm pour un échantillon de profondeur 12 mm; ladite phase aqueuse étant molle ou fluide à 25°C;
une structure principale de phase cristalline rigide comprenant un réseau maillé tridimensionnel ouvert, enchevêtré, de cristaux allongés, diffractant la lumière, d'acide mono- et/ou di-carboxylique neutralisé ayant un diamètre ou une longueur supérieur à 400 nm;
dans lequel ledit pain nettoyant comprenant ladite structure principale de phase cristalline rigide et ladite phase aqueuse possède un indice de pénétration de zéro à environ 12 mm pour un échantillon de profondeur 25 mm de ce pain nettoyant;
dans lequel lesdits indices de pénétration sont mesurés à 25°C à l'aide d'une sonde de pénétromètre pondérée standard de 247 grammes munie d'une aiguille conique fixée sur un axe de 9 pouces (22,9 cm), pesant 47 grammes, avec 200 grammes au sommet de cet axe pour faire un total de 247 grammes, ladite aiguille conique ayant un sommet de 19/32 pouce (1,51 cm) et une pointe de 1/32 pouce (0,08 cm);
dans lequel ledit acide carboxylique neutralisé est choisi dans le groupe constitué par un acide monocarboxylique (savon) et/ou un acide dicarboxylique, neutralisé au lithium et/ou au sodium, et leurs mélanges;
dans lequel ledit acide monocarboxylique possède une chaîne alkyle ou alkylène grasse d'environ 12 à environ 24 atomes de carbone;
dans lequel ledit acide dicarboxylique possède une chaîne alkyle ou alkylène grasse d'environ 12 à environ 18 atomes de carbone; et
dans lequel au moins 80% dudit acide carboxylique possède des chaînes alkyle saturées;
dans lequel ladite structure principale de phase cristalline rigide occupe de 3% à 75% en volume de ce pain nettoyant; et
dans lequel ledit acide carboxylique neutralisé constitue de plus de 5% à 75% en poids de ce pain nettoyant; et
dans lequel ledit pain nettoyant contient de 15% à 94% en poids d'eau.

2. Pain nettoyant selon la revendication 1, dans lequel au moins 80% dudit acide carboxylique répond à la formule générale: dans laquelle:$\text{a + b = 8 à 20}$ chaque a, b = 0 à 20
X = H, OR, R, ou leurs mélanges
R = alkyle en C₁-C₃, H, ou leurs mélanges
M = Na, Li, ou leurs mélanges.

3. Pain nettoyant selon la revendication 2, dans lequel $\text{a + b = 10-16}$ ; chacun desdits a, b = 0-16; X = H, OR; R = H; et M = Na.

4. Pain nettoyant selon la revendication 3, dans lequel lesdits cristaux allongés se composent de savon d'acide gras sodique d'aspect fribreux dont au moins 25% desdites chaînes alkyle grasses saturées sont une seule longueur de chaîne; et dans lequel ledit pain contient: de 15% à 75% en poids dudit savon sodique; dans lequel ledit pain contient un acide carboxylique non neutralisé (libre) à raison de pas plus de 50% en poids dudit savon; et, de préférence, dans lequel ledit pain contient ledit savon sodique et de l'eau; et de 2% à 60% en poids d'un tensioactif synthétique choisi dans le groupe constitué par les alkylsulfates, les paraffinesulfonates, les alkylglycéryléthersulfonates, les acylsarcosinates, les méthylacyltaurates, les alkyl(linéaires)benzènesulfonates, les N-acylglutamates, les alkylglucosides, les esters d'α-sulfo-acides gras, les acyliséthionates, les alkylsulfosuccinates, les alkyléthercarboxylates, les esters alkylphosphates, les esters alkylphosphates éthoxylés, les esters de méthylglucose, les produits de condensation de protéines, les oxydes d'alkylamines, les alkylbétaïnes, les alkylsultaïnes, les alkyléthersulfates comportant 1 à 12 groupes éthoxy, et leurs mélanges, dans lequel lesdits tensioactifs contiennent des chaînes alkyle en C₈-C₂₂.

5. Pain nettoyant selon la revendication 4, dans lequel ledit tensioactif synthétique est hygroscopique; ledit tensioactif hygroscopique étant défini comme étant un tensioactif qui absorbe au moins 20% de son poids sec en eau à 26°C et à 80% d'humidité relative en trois jours, et dans lequel ledit pain est relativement non gonflant; et, de préférence, dans lequel ledit tensioactif hygroscopique est choisi dans le groupe constitué par les esters d'α-sulfo-acides gras; les alkylsulfates; les alkyléthercarboxylates; les alkylbétaïnes; les alkylsultaïnes; les oxydes d'alkylamines; les alkyléthersulfates; et leurs mélanges.

6. Pain nettoyant selon la revendication 4 ou 5, dans lequel le rapport de ladite eau audit savon est d'environ 1:1 à environ 5:1; ladite eau est présente à raison de 25% à 60% en poids; dans lequel ledit savon possède des chaînes alkyle grasses en C₁₄ à C₂₂ et ladite proportion de savon dans ledit pain est de 15% à 35% en poids; dans lequel au moins 85% desdites chaînes alkyle de savon sont saturées; dans lequel ledit acide carboxylique non neutralisé (libre) représente de zéro à environ 25% en poids de ce savon; et dans lequel la proportion de ce tensioactif synthétique est de 4% à 25% en poids du pain et ledit tensioactif est choisi dans le groupe constitué par les acyliséthionates de sodium, les acylsarcosinates de sodium, les esters d'α-sulfo-acides gras de sodium, les paraffinesulfonates de sodium, les alkyléthersulfates de sodium, les alkylsulfates de sodium, les alkyl(linéaires)benzènesulfonates de sodium, les alkylbétaïnes, les alkylsultaïnes et les oxydes de trialkylamines; et de préférence dans lequel ledit rapport de l'eau au savon est d'environ 1,5:1 à environ 2:1; ledit acide carboxylique non neutralisé (libre) représente de zéro à 17% en poids dudit savon; la proportion de ladite eau est de 30% à 45% en poids; ladite chaîne alkyle grasse de savon comporte d'environ 14 à environ 18 atomes de carbone; dans lequel au moins 95% desdites chaînes alkyle sont saturées; la proportion dudit savon est de 15% à 30% en poids; et la proportion dudit tensioactif synthétique est de 8% à 16% en poids.

7. Pain nettoyant selon la revendication 5 ou 6, dans lequel ledit pain contient de 0,1% à 40% en poids d'une matière hydrophobe choisie dans le groupe constitué par: la cire microcristalline, la vaseline, la cire de carnauba, la cire de palme, la cire de candelilla, la cire de canne à sucre, les triglycérides végétaux, la cire d'abeille, le blanc de baleine, la lanoline, la cire de bois, la cire de shellac, les triglycérides animaux, la cire minérale, l'ozocérite, la cérésine et la cire de Fischer-Tropsch; et de préférence dans lequel ledit pain contient de 2% à 35% en poids de ladite matière hydrophobe, choisie dans le groupe constitué par la vaseline et la cire, ladite vaseline et ladite cire, et leurs mélanges, ayant un point de fusion d'environ 49°C (120°F) à environ 85°C (185°F); et mieux encore dans lequel ledit pain comprend de 5% à 25%_{,} en poids du pain, de cire de paraffine; et dans lequel ledit pain contient de 1% à 50% en poids d'une matière organique non ionique, non volatile, soluble dans l'eau, ayant une solubilité d'au moins 5 parties dans 10 parties d'eau; et dans lequel ladite matière organique soluble dans l'eau est choisie dans le groupe constitué par un polyol de structure: dans laquelle R₁ = H, alkyle en C₁-C₄; R₂ = H CH₃; et n = 1-200;
les alcane-diols en C₂-C₁₀; le sorbitol; la glycérine; les sucres; les dérivés de sucres; l'urée; et
les éthanolamines de structure générale (HOCH₂CH₂)ₓNH_{y}, dans laquelle x = 1-3; y = 0-2; et $\text{x + y = 3}$ , et leurs mélanges; et de préférence dans lequel la matière organique non ionique, non volatile, soluble dans l'eau, constitue de 5% à 20% en poids du pain; ladite matière organique est choisie dans le groupe constitué par le propylèneglycol, la glycérine, le saccharose et l'urée, et leurs mélanges.

8. Pain nettoyant selon la revendication 5, 6 ou 7, dans lequel ledit pain contient ledit savon de sodium, ladite eau et ledit tensioactif synthétique et de 0,1% à 70% en poids d'autres ingrédients choisis dans le groupe constitué par:
de 1% à 10% en poids de savon de potassium;
de 1% à 35% en poids de savon de magnésium;
de 1% à 35% en poids de savon de calcium;
de 1% à 15% en poids de savon de triéthanolammonium;
de 1% à 60% en poids de matières impalpables insolubles dans l'eau, choisies dans le groupe constitué par le carbonate de calcium et le talc;
de 0,1% à 20% en poids d'un émollient polymère;
de 0,5% à 25% en poids d'une argile aluminosilicate et/ou d'autres argiles; dans lequel lesdits aluminosilicates et lesdites argiles sont choisis dans le groupe constitué par les zéolithes; le kaolin, la kaolinite, la montmorillonite, l'attapulgite, l'illite, la bentonite, l'halloysite, et les argiles calcinées;
de 1% à 50% en poids de sel et d'hydrates de sels; et leurs mélanges; et dans lequel ledit sel et hydrate de sel possède un cation choisi dans le groupe constitué par: le sodium, le potassium, le magnésium, le calcium, l'aluminium, le lithium, l'ammonium, le monoéthanolammonium, le diéthanolammonium et le triéthanolammonium; et dans lequel ledit sel et hydrate de sel possèdent un anion choisi dans le groupe constitué par: le chlorure, le bromure, le sulfate, le métasilicate, l'orthophosphate, le pyrophosphate, le polyphosphate, le métaborate, le tétraborate, le carbonate, le bicarbonate, l'hydrogénophosphate, le méthylsulfate et les mono- et poly-carboxylates de 6 atomes de carbone ou moins.

9. Procédé de fabrication d'un pain nettoyant selon les revendications 1 à 8, ledit procédé comprenant les étapes qui consistent à:
I. former un liquide fondu aqueux comprenant de 20% à 94% en poids d'eau et d'environ plus de 5% à 75%, en poids du pain, dudit acide carboxylique neutralisé;
II. verser ledit liquide fondu dans un moule à savon en forme de pain; et
III. cristalliser ledit liquide fondu moulé en refroidissant pour obtenir ledit pain nettoyant; de préférence
dans lequel le liquide fondu aqueux est préparé par neutralisation d'un mélange aqueux dudit acide carboxylique avec un hydroxyde choisi dans le groupe constitué par l'hydroxyde de sodium ou l'hydroxyde de lithium, et leurs mélanges, sous agitation à une température d'environ 50°C (120°F) à environ 95°C (205°F); et ledit liquide fondu contient de 2% à 15%_{,} en poids dudit pain, d'un "sel favorisant la cristallisation" choisi dans le groupe constitué par un sel de sodium ou de lithium sulfate, chlorure acétate et citrate, et leurs mélanges; et de préférence, lorsque ladite phase aqueuse de liquide fondu aqueux contient de 2% à 40% d'un auxiliaire de solubilisation, ledit auxiliaire de solubilisation est choisi dans le groupe constitué par:
(a) les solvants organiques non ioniques, non volatils, solubles dans l'eau, choisis dans le groupe constitué par un polyol de structure: dans laquelle R₁ = H, alkyle en C₁-C₄; R₂ = H, CH₃; et n = 1-200;
les alcane-diols en C₂-C₁₀; le sorbitol; la glycérine; les sucres; les dérivés de sucres; l'urée; et les éthanolamines de structure générale (HOCH₂CH₂)ₓNH_{y}, dans laquelle x = 1-3; y = 0-2; et $\text{x + y = 3}$ ;
(b) les alcools de 1 à 5 atomes de carbone;
(c) un tensioactif synthétique choisi dans le groupe constitué par les alkylsulfates, les paraffinesulfonates, les alkylglycéryléthersulfonates, les acylsarcosinates anioniques, les méthylacyltaurates, les alkyl(linéaires)benzènesulfonates, les N-acylglutamates, les alkylglucosides, les esters d'α-sulfo-acides gras, les acyliséthionates, les alkylsulfosuccinates, les alkyléthercarboxylates, les esters alkylphosphates, les esters alkylphosphates éthoxylés, les esters de méthylglucose, les produits de condensation de protéines, les oxydes d'alkylamines, les alkylbétaïnes, les alkylsultaïnes, les alkyléthersulfates comportant 1 à 12 groupes éthoxy, et leurs mélanges, dans lequel lesdits tensioactifs contiennent des chaînes alkyle en C₈-C₂₂; et
leurs mélanges; et
dans lequel ledit auxiliaire de solubilisation est ajouté pour augmenter la proportion dudit acide carboxylique neutralisé dissous dans ladite phase aqueuse fondue continue dans l'étape I.

10. Procédé selon la revendication 9, dans lequel ladite phase aqueuse contient de 20% à 100% d'eau, en poids de ladite phase aqueuse; et dans lequel ladite phase cristalline rigide contient de 75% à 100% dudit acide carboxylique neutralisé, en poids de ladite phase cristalline; et dans lequel ledit pain possède un indice de pénétration de 3 mm à 9 mm pour ledit échantillon de savon de 25 mm.

11. Composition de pain nettoyant pour la toilette selon la revendication 1, comprenant un réseau maillé cristallin tridimensionnel ouvert, enchevêtré, rigide, de cristaux de savon de sodium allongés ayant un diamètre ou une longueur supérieure à 400 nm; ledit pain de savon comprenant: de 15% à 50% en poids de savon d'acide gras de sodium composé d'au moins 50% de chaînes alkylène grasses saturées comportant 12-24 atomes de carbone, dont au moins 25% desdites chaînes alkyle grasses saturées ont une seule longueur de chaîne; de 15% à 60% en poids d'eau; et de 2% à 60% en poids d'un tensioactif synthétique hygroscopique, dans lequel ledit tensioactif synthétique hygroscopique est choisi parmi les tensioactifs qui absorbent au moins 20% de leur poids sec en eau 26°C et à 80% d'humidité relative en trois jours.

12. Pain nettoyant pour la toilette selon la revendication 11, dans lequel ledit tensioactif synthétique hygroscopique est choisi dans le groupe constitué par les esters d'α-sulfo-acides gras; les alkylsulfates; les alkyléthercarboxylates; les alkylbétaïnes; les alkylsultaïnes; les oxydes d'alkylamines; les alkyléthersulfates; et leurs mélanges; et dans lequel ledit pain contient de 0,5% à 40% en poids de sels et/ou d'hydrates de sels choisis dans le groupe constitué par le chlorure de sodium, le sulfate de sodium, l'hydrogénophosphate disodique, le pyrophosphate de sodium, le tétraborate de sodium, l'acétate de sodium, le citrate de sodium, et d'autres sels compatibles d'acides minéraux et d'acides organiques à chaîne courte.
